



US010423084B2

(12) **United States Patent**  
Aichi et al.

(10) **Patent No.:** US 10,423,084 B2  
(45) **Date of Patent:** Sep. 24, 2019

(54) **METHOD FOR PRODUCING LIQUID DEVELOPER**(71) Applicant: **CANON KABUSHIKI KAISHA**,  
Tokyo (JP)(72) Inventors: **Yasuhiro Aichi**, Tokyo (JP); **Junji Ito**,  
Hiratsuka (JP); **Jun Shirakawa**,  
Kawaguchi (JP); **Waka Hasegawa**,  
Tokyo (JP); **Ryo Natori**, Tokyo (JP);  
**Ayano Mashida**, Kawasaki (JP)(73) Assignee: **CANON KABUSHIKI KAISHA**,  
Tokyo (JP)

(\* ) Notice: Subject to any disclaimer, the term of this patent is extended or adjusted under 35 U.S.C. 154(b) by 0 days.

(21) Appl. No.: 16/190,237

(22) Filed: Nov. 14, 2018

(65) **Prior Publication Data**

US 2019/0155180 A1 May 23, 2019

(30) **Foreign Application Priority Data**Nov. 20, 2017 (JP) ..... 2017-222664  
Jul. 6, 2018 (JP) ..... 2018-129132(51) **Int. Cl.**G03G 9/08 (2006.01)  
G03G 9/125 (2006.01)  
G03G 9/13 (2006.01)(52) **U.S. Cl.**

CPC ..... G03G 9/0804 (2013.01); G03G 9/125 (2013.01); G03G 9/132 (2013.01)

(58) **Field of Classification Search**CPC ..... G03G 9/0804; G03G 9/125; G03G 9/132  
USPC ..... 430/114, 137.22

See application file for complete search history.

(56)

**References Cited**

## U.S. PATENT DOCUMENTS

|              |         |                |
|--------------|---------|----------------|
| 5,760,257 A  | 6/1998  | Tanaka et al.  |
| 7,833,687 B2 | 11/2010 | Kato et al.    |
| 8,399,170 B2 | 3/2013  | Iwase et al.   |
| 8,697,327 B2 | 4/2014  | Shibata et al. |
| 8,722,302 B2 | 5/2014  | Maeda et al.   |
| 8,815,484 B2 | 8/2014  | Tanaka et al.  |
| 9,057,970 B2 | 6/2015  | Ida et al.     |
| 9,229,345 B2 | 1/2016  | Ikeda et al.   |

(Continued)

## FOREIGN PATENT DOCUMENTS

|                |         |  |
|----------------|---------|--|
| CA 2 609 825   | 11/2006 |  |
| JP 2003-241439 | 8/2003  |  |

(Continued)

## OTHER PUBLICATIONS

U.S. Appl. No. 16/140,615, Waka Hasegawa, filed Sep. 25, 2018.

Primary Examiner — Mark A Chapman

(74) Attorney, Agent, or Firm — Venable LLP

(57) **ABSTRACT**

A method for producing a liquid developer, the method including a step of producing a toner particle by applying a shear force to a mixture of a polyester resin A and B, and a toner particle dispersing agent in a liquid a, wherein the polyester resin A has a number-average molecular weight from 3,000 to 7,000, an acid value of at least 5, and a carboxy group; the polyester resin B has a number-average molecular weight from 4,000 to 20,000 and an acid value of not more than 2; the toner particle dispersing agent has a primary amino group and an amine value of at least 40; the mass ratio (B/(A+B)) for the polyester resin B is 0.3 to 0.9; and the following relationship is satisfied: SP value of liquid a<SP value of the toner particle dispersing agent<SP value of polyester resin B.

**11 Claims, 2 Drawing Sheets**

---

| (56)                     | References Cited        |                 |                         |  |
|--------------------------|-------------------------|-----------------|-------------------------|--|
| U.S. PATENT DOCUMENTS    |                         |                 |                         |  |
| 9,348,247 B2             | 5/2016 Ida et al.       | 2017/0102628 A1 | 4/2017 Kabashima et al. |  |
| 9,556,290 B2             | 1/2017 Nishiura et al.  | 2018/0046105 A1 | 2/2018 Tanabe et al.    |  |
| 9,715,187 B2             | 7/2017 Mukumoto et al.  | 2018/0046106 A1 | 2/2018 Shirakawa et al. |  |
| 9,740,118 B2             | 8/2017 Hasegawa et al.  | 2018/0059566 A1 | 3/2018 Tanabe et al.    |  |
| 9,766,568 B2             | 9/2017 Ito et al.       | 2018/0143546 A1 | 5/2018 Hasegawa et al.  |  |
| 9,857,716 B2             | 1/2018 Natori et al.    | 2018/0329333 A1 | 11/2018 Tokunaga et al. |  |
| 9,880,482 B2             | 1/2018 Hasegawa et al.  | 2018/0348658 A1 | 12/2018 Tsuchida et al. |  |
| 9,891,546 B2             | 2/2018 Ito et al.       |                 |                         |  |
| 9,891,547 B2             | 2/2018 Tanabe et al.    | JP 3718915      | 11/2005                 |  |
| 9,897,936 B2             | 2/2018 Natori et al.    | JP 2014-232211  | 12/2014                 |  |
| 9,971,268 B2             | 5/2018 Tanabe et al.    | JP 2016-224405  | 12/2016                 |  |
| 2010/0136474 A1          | 6/2010 Iwase et al.     | WO 2006/126566  | 11/2006                 |  |
| 2014/0356779 A1          | 12/2014 Hasegawa et al. | WO 2007/000974  | 1/2007                  |  |
| 2014/0377697 A1          | 12/2014 Nishiura et al. | WO 2007/000975  | 1/2007                  |  |
| 2015/0004539 A1          | 1/2015 Watanabe et al.  | WO 2007/108485  | 9/2007                  |  |
|                          |                         | WO 2009/041634  | 4/2009                  |  |
| FOREIGN PATENT DOCUMENTS |                         |                 |                         |  |



Fig. 1

**Fig. 2**

## 1

## METHOD FOR PRODUCING LIQUID DEVELOPER

## BACKGROUND OF THE INVENTION

## Field of the Invention

The present invention relates to the liquid developer that is used in image-forming apparatuses that employ an electrophotographic system, e.g., electrophotography, electrostatic recording, electrostatic printing, and so forth.

## Description of the Related Art

Plate-based presses have in the past been used to produce printed materials for which a certain number of copies are required, such as regional advertising, internally distributed business documents, and large posters.

In place of these conventional presses, on-demand printers have entered into use in recent years; these on-demand printers can rapidly respond to a diversifying range of needs and support inventory reductions. Electrophotographic printers that use liquid developers and inkjet printers capable of high speeds and high quality printing are anticipated for such on-demand printers.

Liquid developers use an electrically insulating liquid as a carrier liquid and because of this are more resistant than dry developers to the problem of aggregation of the toner particles in the liquid developer during storage, and thus enable the use of microfine toner particles. As a result, liquid developers provide a better fine line image reproducibility and a better gradation reproducibility than dry developers and exhibit an excellent color reproducibility and also excellence in high-speed image-forming methods. Development is becoming quite active with regard to high-image-quality, high-speed digital printing apparatuses that exploit these excellent characteristics by using liquid developers. In view of these circumstances, there is demand for the development of liquid developers that have even better properties.

Photocurable liquid developers are known within the sphere of liquid developers. A photocurable liquid developer uses a reactive functional group-bearing monomer or oligomer as the electrical insulating liquid and can be prepared by the addition and dissolution of a photopolymerization initiator. This photocurable liquid developer is cured by a polymerization reaction when exposed to light, e.g., ultraviolet radiation, and can accommodate high-speed development processing.

A method is already known, for example, as in Japanese Patent Application Laid-open No. 2016-224405, for producing a microfine toner particle using the combination of a resin B having an acid value and a resin A bearing an alkali metal sulfonate salt group or an alkaline-earth metal sulfonate salt group.

With regard to methods for producing a liquid developer that exhibits an excellent toner particle dispersion stability and excellent charging characteristics on the part of the liquid developer, a method is known, as in WO 09/041634, for producing a toner particle by a coacervation technique in the presence of a special toner particle dispersing agent and a resin having an acid value.

The liquid developers produced using these methods do have excellent initial characteristics as developers. However, when the residual undeveloped toner particles and the residual untransferred toner particles at, e.g., the developing roller and photosensitive member, are recovered using a cleaning blade, and when recovery continues for a certain

## 2

amount of time, the recovered toner particles can aggregate and aggregates can then end up being produced.

In order to inhibit this toner particle aggregation, an art is disclosed in Japanese Patent Application Laid-open No. 2014-232211 wherein core particles and shell particles are separately prepared; a toner particle is then prepared by attaching the shell particles to the circumference of the core particle; and a basic dispersing agent is also added.

## SUMMARY OF THE INVENTION

A microfine toner particle can be produced when a toner particle dispersing agent is used during toner particle production; however, when the toner particle dispersing agent is not tightly bonded to the toner particle surface, aggregates may be produced when shear force is input from, for example, the cleaning blade. Moreover, when a basic toner particle dispersing agent is added post-toner particle production, the basic toner particle dispersing agent can separate from the toner particle and the resistance of the insulating liquid carrier may then be reduced.

By bringing about an efficient orientation and tight bonding of the basic toner particle dispersing agent to the toner particle surface, the present invention provides a method for producing a liquid developer that is resistant to reductions in the volume resistivity of the insulating liquid carrier, that can resist the production of aggregates even when shear force is applied to the toner particle by, e.g., the cleaning blade, and that exhibits an excellent toner particle dispersion stability.

The present invention is a method for producing a liquid developer containing an insulating liquid carrier, a toner particle dispersing agent, and a toner particle that contains a polyester resin A and a polyester resin B, the method including the following process A or process B: the process

30 A having a step of particulating a mixture of the polyester resin A, the polyester resin B, and the toner particle dispersing agent in a liquid a by applying a shear force to the mixture, and a step of producing a toner particle in the liquid a via a molten state; and the process B having a step of 35 dissolving, in a solvent b, a mixture of the polyester resin A, the polyester resin B, and the toner particle dispersing agent, a step of mixing the resulting solution with the liquid a and applying shear force to particulate the mixture in the liquid a and provide a toner particle, and a step of distillatively 40 removing the solvent b, wherein the liquid a dissolves the toner particle dispersing agent and does not dissolve the polyester resin A and does not dissolve the polyester resin B, the polyester resin A has a number-average molecular weight from 3,000 to 7,000, the polyester resin A has an acid 45 value of at least 5 mg KOH/g, the polyester resin A has, as an acidic group, a carboxy group deriving from trimellitic acid and/or trimellitic anhydride, the polyester resin B has a number-average molecular weight from 4,000 to 20,000, the polyester resin B has an acid value of not more than 2 mg KOH/g, the toner particle dispersing agent has a primary 50 amino group, the toner particle dispersing agent has an amine value of at least 40 mg KOH/g, a mass ratio (B/(A+B)) of the polyester resin B to a sum of the polyester resin A and the polyester resin B is from 0.3 to 0.9, and an SP value of the liquid a, an SP value of the polyester resin B, and an SP value of the toner particle dispersing agent satisfy 55 the following relationship: SP value of liquid a < SP value of toner particle dispersing agent < SP value of polyester resin B.

Thus, by bringing about an efficient orientation and tight bonding of the basic toner particle dispersing agent to the toner particle surface, the present invention provides a

60

method for producing a liquid developer that is resistant to reductions in the volume resistivity of the insulating liquid carrier, that can resist the production of aggregates even when shear force is applied to the toner particle by, e.g., the cleaning blade, and that exhibits an excellent toner particle dispersion stability.

Further features of the present invention will become apparent from the following description of exemplary embodiments with reference to the attached drawings.

#### BRIEF DESCRIPTION OF THE DRAWINGS

FIG. 1 is a schematic diagram of a developing apparatus; and

FIG. 2 is a schematic diagram of a developing apparatus.

#### DESCRIPTION OF THE EMBODIMENTS

The present invention is a method for producing a liquid developer containing an insulating liquid carrier, a toner particle dispersing agent, and a toner particle that contains a polyester resin A and a polyester resin B, the method including the following process A or process B: the process A having a step of particulating a mixture of the polyester resin A, the polyester resin B, and the toner particle dispersing agent in a liquid a by applying a shear force to the mixture, and a step of producing a toner particle in the liquid a via a molten state; and the process B having a step of dissolving, in a solvent b, a mixture of the polyester resin A, the polyester resin B, and the toner particle dispersing agent, a step of mixing the resulting solution with the liquid a and applying shear force to particulate the mixture in the liquid a and provide a toner particle, and a step of distillatively removing the solvent b, wherein the liquid a dissolves the toner particle dispersing agent and does not dissolve the polyester resin A and does not dissolve the polyester resin B, the polyester resin A has a number-average molecular weight from 3,000 to 7,000, the polyester resin A has an acid value of at least 5 mg KOH/g, the polyester resin A has, as an acidic group, a carboxy group deriving from trimellitic acid and/or trimellitic anhydride, the polyester resin B has a number-average molecular weight from 4,000 to 20,000, the polyester resin B has an acid value of not more than 2 mg KOH/g, the toner particle dispersing agent has a primary amino group, the toner particle dispersing agent has an amine value of at least 40 mg KOH/g, a mass ratio (B/(A+B)) of the polyester resin B to a sum of the polyester resin A and the polyester resin B is from 0.3 to 0.9, and an SP value of the liquid a, an SP value of the polyester resin B, and an SP value of the toner particle dispersing agent satisfy the following relationship: SP value of liquid a<SP value of toner particle dispersing agent<SP value of polyester resin B.

Unless specifically indicated otherwise, the expressions "from XX to YY" and "XX to YY" that show numerical value ranges refer in the present invention to numerical value ranges that include the lower limit and upper limit that are the end points.

#### Materials

The materials used in and by the present invention are described in detail herebelow.

#### Liquid a

The toner particle is produced in a liquid a in the production method according to the present invention.

The liquid a satisfies the following relationship for the SP value of the liquid a, the SP value of the polyester resin B, and the SP value of the toner particle dispersing agent: SP

value of liquid a<SP value of toner particle dispersing agent<SP value of polyester resin B.

In addition, the liquid a dissolves the toner particle dispersing agent and does not dissolve the polyester resin A and B. Otherwise, the liquid a may be any medium that can transmit the shear force applied in the process A to the mixture of polyester resin A+polyester resin B+toner particle dispersing agent.

The criterion for "the liquid a does not dissolve a polyester resin" is that not more than 1 mass parts of the polyester resin dissolves in 100 mass parts of the liquid a at a temperature of 25° C. The criterion for "the liquid a dissolves the toner particle dispersing agent" is that at least 10 mass parts of the toner particle dispersing agent dissolves in 100 mass parts of the liquid a at a temperature of 25° C. Preferably the liquid a does not dissolve the toner particle. The criterion for "the liquid a does not dissolve the toner particle" is that not more than 1 mass parts of the toner particle dissolves in 100 mass parts of the liquid a at a temperature of 25° C.

Considering the general range of SP values for polyester resins and toner particle dispersing agents, an organic solvent having a low SP value is preferably used for the liquid a.

The liquid a can be exemplified by hydrocarbon solvents such as hexane, octane, isooctane, decane, isodecane, decalin, nonane, dodecane, and isododecane; paraffin solvents such as Isopar E, Isopar G, Isopar H, Isopar L, Isopar M, and Isopar V (ExxonMobil), Shellsol A100 and Shellsol A150 (Shell Chemicals Japan Ltd.), and Moresco White MT-30P (Matsumura Oil Co., Ltd.); and substituent-bearing hydrocarbons. For example, hexane and Moresco White MT-30P are preferred. A single one or a mixture of these can be used.

The liquid a preferably contains a cationically polymerizable liquid monomer. Specific examples here are cyclic ether monomers such as epoxides and oxetanes and vinyl ether compounds.

This vinyl ether compound refers to a compound having the vinyl ether structure ( $-\text{CH}=\text{CH}-\text{O}-\text{C}-$ ).

Specific examples are dodecyl vinyl ether, dicyclopentadiene vinyl ether, cyclohexanediethanol divinyl ether, tricyclodecane vinyl ether, dipropylene glycol divinyl ether, trimethylolpropane trivinyl ether, 2-ethyl-1,3-hexanediol divinyl ether, 2,4-diethyl-1,5-pentanediol divinyl ether, 2-butyl-2-ethyl-1,3-propanediol divinyl ether, neopentyl glycol divinyl ether, pentaerythritol tetravinyl ether, and 1,2-decanediol divinyl ether.

After the toner particle has been produced, the liquid a as such may be used as the carrier liquid for the liquid developer, or it may be replaced, e.g., by decantation or filtration, by an insulating liquid carrier suitable for liquid developers. The liquid a as such is preferably used as the carrier liquid for the liquid developer after the toner particle has been produced. That is, the liquid a is preferably an insulating liquid carrier.

#### Toner Particle

From the standpoint of obtaining a high-definition image, the toner particle has a 50% particle diameter on a volume basis (D50) preferably from 0.05  $\mu\text{m}$  to 2.0  $\mu\text{m}$ , more preferably from 0.05  $\mu\text{m}$  to 1.2  $\mu\text{m}$ , and still more preferably from 0.05  $\mu\text{m}$  to 1.0  $\mu\text{m}$ .

When the 50% particle diameter on a volume basis (D50) of the toner particle is in the indicated range, the resolution and image density of the toner image formed by the liquid developer can be brought to satisfactorily high levels, and at the same time the film thickness of the toner image can be made satisfactorily thin.

An example of the process A in the toner particle production method is the execution of a heating/stirring method subsequent to a method such as a known wet pulverization procedure. The details of the wet pulverization procedure are described in, for example, WO 2006/126566 and WO 2007/108485. The heating/stirring method may be any such method that provides—via a molten state wherein the molecules constituting the particles yielded by pulverization can move freely—an energetically stable state, and that can provide stirring to a degree that prevents sedimentation and aggregation of the molten particles.

The toner particle concentration in the liquid developer may be brought to from about 1 mass % to 50 mass % and is preferably from 2 mass % to 40 mass %.

The process B in the toner particle production method can be exemplified by known methods, for example, the coacervation method. The details of the coacervation method are described in, for example, Japanese Patent Application Laid-open No. 2003-241439, WO 2007/000974, and WO 2007/000975. Known methods such as these may be used in the present invention.

The toner particle concentration in the liquid developer may be brought to from about 1 mass % to 50 mass % and is preferably from 2 mass % to 40 mass %.

The toner particle contains a polyester resin A and a polyester resin B.

#### Polyester Resin

Polyester resin A and polyester resin B are used as binder resins for the toner particle. To the extent that the effects of the present invention are not impaired, a resin known for use as a binder resin may be used in addition to polyester resin A and polyester resin B.

The polyester resin is preferably provided by the condensation polymerization of an alcohol monomer and a carboxylic acid monomer.

The alcohol monomer can be exemplified by the following: alkylene oxide adducts on bisphenol A, e.g., polyoxypropylene(2.2)-2,2-bis(4-hydroxyphenyl)propane, polyoxypropylene(3.3)-2,2-bis(4-hydroxyphenyl)propane, polyoxyethylene(2.0)-2,2-bis(4-hydroxyphenyl)propane, polyoxypropylene(2.0)-2,2-bis(4-hydroxyphenyl)propane, polyoxypropylene(2.0)-polyoxyethylene(2.0)-2,2-bis(4-hydroxyphenyl)propane, and polyoxypropylene(6)-2,2-bis(4-hydroxyphenyl)propane, as well as ethylene glycol, diethylene glycol, triethylene glycol, 1,2-propanediol, 1,3-propanediol, 1,4-butanediol, neopentyl glycol, 1,4-butanediol, 1,5-pentanediol, 1,6-hexanediol, 1,4-cyclohexanedimethanol, dipropylene glycol, polyethylene glycol, polypropylene glycol, polytetramethylene glycol, bisphenol A, hydrogenated bisphenol A, glycerol, sorbitol, 1,2,3,6-hexanetetrol, 1,4-sorbitan, pentaerythritol, dipentaerythritol, tripentaerythritol, 1,2,4-butanetriol, 1,2,5-pentanetriol, 2-methylpropanetriol, 2-methyl-1,2,4-butanetriol, trimethylolethane, trimethylolpropane, and 1,3,5-trihydroxymethylbenzene.

The carboxylic acid monomer, on the other hand, can be exemplified by the following:

aromatic dicarboxylic acids such as phthalic acid, isophthalic acid, and terephthalic acid and their anhydrides; alkyl dicarboxylic acids such as succinic acid, adipic acid, sebacic acid, and azelaic acid and their anhydrides; succinic acid substituted by an alkyl group having 6 to 18 carbons or by an alkenyl group having 6 to 18 carbons, and anhydrides thereof; and unsaturated dicarboxylic acids such as fumaric acid, maleic acid, and citraconic acid and their anhydrides.

The following monomers can be used in addition to the preceding: polyhydric alcohols such as the oxyalkylene

ethers of novolac-type phenolic resins; and polybasic carboxylic acids such as trimellitic acid, pyromellitic acid, benzophenonetetracarboxylic acid, and their anhydrides.

Among the preceding, preferably either the carboxylic acid monomer or the alcohol monomer contains an aromatic ring. The presence of the aromatic ring causes a reduction in the crystallinity of the polyester resin and can thereby improve the solubility in solvent.

Among the preceding, the at least two species of polyester resin A and polyester resin B are used in the following ratio.

The mass ratio (B/(A+B)) of the polyester resin B to the sum of the polyester resin A and the polyester resin B must be from 0.3 to 0.9. From 0.4 to 0.8 is preferred.

#### Polyester Resin A

By selecting a polyester resin A as described in the following, a toner can be produced in which the toner particle dispersing agent is tightly bonded to the toner particle.

The number-average molecular weight of the polyester resin A is from 3,000 to 7,000 and is more preferably from 4,000 to 7,000. The polyester resin A is used in order to strongly adsorptively interact with the toner particle dispersing agent. The elution of the toner particle dispersing agent into the insulating liquid carrier can be inhibited when the number-average molecular weight is at least 3,000, while control of the particle diameter of the toner particle is facilitated when the number-average molecular weight is not more than 7,000.

The polyester resin A has an acid value of at least 5 mg KOH/g and contains, as an acidic group, a carboxy group derived from trimellitic acid or trimellitic anhydride.

It was found that a carboxy group derived from trimellitic acid or trimellitic anhydride exhibits a strong adsorptive interaction with the primary amino group present in the toner particle dispersing agent. It is therefore thought that the production of a toner particle in which the toner particle dispersing agent is tightly bonded to the polyester resin A present in the toner particle is made possible when such a carboxy group is present and the acid value is at least 5 mg KOH/g.

This carboxy group is preferably present in terminal position (more preferably in main chain terminal position) on the polyester resin A. The presence in terminal position enables bonding to occur with the amino group in the toner particle dispersing agent under conditions of low steric hindrance, thus enabling a multipoint adsorption and further raising the inhibitory effect on toner particle aggregation. The acid value is preferably at least 5 mg KOH/g and is more preferably at least 10 mg KOH/g. The upper limit, on the other hand, is not particularly limited, but is generally not more than 30 mg KOH/g and is preferably not more than 25 mg KOH/g.

#### Polyester Resin B

The polyester resin B is incorporated in the toner particle; preferably substantially does not interact with the toner particle dispersing agent described below; and is selected to have an SP value higher than the SP values of the liquid a and the toner particle dispersing agent. Thus, the following is satisfied: SP value of liquid a < SP value of toner particle dispersing agent < SP value of polyester resin B. This facilitates the entry of the polyester resin B into the interior of the toner particle. It is thought that, as a result, orientation of the toner particle dispersing agent and the polyester resin A, while residing in a state of adsorptive interaction, to the toner particle surface is facilitated and a toner exhibiting an excellent dispersion stability can be produced.

The following is preferably satisfied: SP value of liquid a+2.0<SP value of toner particle dispersing agent<SP value of polyester resin B-0.5.

The number-average molecular weight of the polyester resin B is from 4,000 to 20,000 and is preferably from 7,000 to 20,000. Elution into the insulating liquid carrier can be suppressed by having the number-average molecular weight of polyester resin B be at least 4,000, while control of the particle diameter of the toner particle is facilitated by having the number-average molecular weight be not more than 20,000.

The polyester resin B has an acid value of not more than 2 mg KOH/g. An acid value of not more than 2 mg KOH/g serves to restrain the inhibition of bond formation between the polyester resin A and the toner particle dispersing agent and is thus preferred. While the lower limit is not particularly limited, it is preferably equal to or greater than 0 mg KOH/g.

The polyester resin B preferably has a sulfo group that has formed a salt with at least one element selected from the group consisting of alkali metals and alkaline-earth metals. In the case of a salt with an alkali metal, this group is represented by  $-\text{SO}_3\text{R}_a$  ( $\text{R}_a$  is an alkali metal element); in the case of a salt with an alkaline-earth metal, this group is represented by  $=(\text{SO}_3)\text{R}_b$  ( $\text{R}_b$  is an alkaline-earth metal element). This group is more preferably a salt with an alkali metal and is still more preferably the sodium salt ( $-\text{SO}_3\text{Na}$ ). The presence of such a sulfo group can bring about stabilization of the polarization of the charge of the moiety where the primary amino group in the toner particle dispersing agent engages in strong adsorptive interaction with the carboxy group in the polyester resin A deriving from trimellitic acid and/or trimellitic anhydride. It is thought that as a consequence the toner particle can more tightly bond with the toner particle dispersing agent and a better aggregation-inhibiting effect is then be obtained.

For example, the synthesis of polyester resin using monomer bearing such a sulfo group can then introduce, into the polyester resin B, a sulfo group formed into a salt with at least one element selected from the group consisting of alkali metals and alkaline-earth metals. An example of the method for this is the use of monosodium 5-sulfoisophthalate or a derivative thereof for the dicarboxylic acid monomer.

From 0.2 mass % to 2.0 mass % is preferred for the content, in the total monomer unit constituting the polyester resin B, of monomer unit deriving from monomer having a sulfo group that has formed a salt with at least one element selected from the group consisting of alkali metals and alkaline-earth metals. Here, "monomer unit" refers to the reacted form of the monomer substance in the polymer.

The mass ratio (B/(A+B)) of the polyester resin B to the sum of the polyester resin B and the polyester resin A is from 0.3 to 0.9 and is preferably from 0.4 to 0.8.

The following is thought to occur when this mass ratio is in the indicated range: the polyester resin B then enters the interior of the toner in the requisite amount and formation of the bonded species of the toner particle dispersing agent bonded to the toner particle surface is facilitated; due, in combination with this, to the strong adsorption of the toner particle dispersing agent to the toner particle under the effect of the polyester resin A, reductions in the resistance of the insulating liquid carrier are then suppressed and the particle aggregation-inhibiting effect of the present invention is also obtained.

#### Toner Particle Dispersing Agent

A toner particle dispersing agent bearing a primary amino group is used in the method according to the present invention for producing a liquid developer. This primary amino group denotes a group represented by  $-\text{NH}_2$ . A liquid developer that exhibits a high dispersion stability can be provided through the use of such a toner particle dispersing agent.

With the goal of causing the appearance of an adequate 10 repulsive force in the carrier liquid, a toner particle dispersing agent may be provided with a substituent for raising the solubility in the carrier liquid. This functions to improve the dispersion stability of the toner particle. On the other hand, a toner particle dispersing agent bearing a primary amino 15 group readily bonds with the polyester resin A. As a consequence, release of the toner particle dispersing agent into the carrier in the absence of adsorption to the toner particle can be suppressed and an excellent dispersion stability is provided and reductions in the resistivity of the liquid developer can be inhibited.

The primary amino group-bearing toner particle dispersing agent is preferably a primary amino group-bearing polymer, and a polyallylamine derivative is preferred. The primary amino group-bearing polymer preferably is not a 25 polymer that has the primary amino group only in terminal position on the polymer main chain. However, it may have the primary amino group in terminal position as long as it has the primary amino group in a position other than terminal position on the polymer main chain.

In addition, it was found that the bond strength between 30 a polyester resin A having the specified acid value and a polymer bearing a primary amino group in a position other than terminal position on the polymer main chain, is significantly stronger than for a polymer bearing a primary 35 amino group only in terminal position on the polymer main chain and for a polymer bearing a secondary or tertiary amino group.

The primary amino group-bearing polymer preferably is a 40 polymer that contains the monomer unit represented by the following formula (1) and the monomer unit represented by 45 the following formula (2). In addition, this primary amino group-bearing polymer has the monomer unit represented by formula (1) in a position other than terminal position on the main chain. That is, polymer having the primary amino group only in terminal position on the polymer main chain is not included. However, the monomer unit with formula (1) may be present in terminal position on the polymer main 50 chain as long as the monomer unit with formula (1) is present at a position other than terminal position on the main chain.

In addition, the amine value deriving from the primary 55 amino group present in the monomer unit represented by formula (1) is preferably at least 50% of the amine value of the primary amino group-bearing polymer.



[In formula (1), K represents a monomer unit having a primary amino group.]

[In formula (2), Q represents a monomer unit that has a possibly substituted alkyl group having at least 6 carbons, a possibly substituted cycloalkyl group having at least 6 carbons, a possibly substituted alkylene group having at least 6 carbons, or a possibly substituted cycloalkylene group having at least 6 carbons.]

The possibly substituted alkyl group having at least 6 carbons and the possibly substituted cycloalkyl group hav-

ing at least 6 carbons encompassed by Q in formula (2) are represented, respectively, by the straight-chain  $—C_nH_{2n+1}$  and the cyclic  $—C_nH_{2n-1}$  and denote alkyl groups and cycloalkyl groups in which the number of carbons n is at least 6. In addition, the possibly substituted alkylene group having at least 6 carbons and the possibly substituted cycloalkylene group having at least 6 carbons are represented, respectively, by the straight-chain  $—C_nH_{2n—}$  and the cyclic  $—C_nH_{2n-2—}$  and denote alkylene groups and cycloalkylene groups in which the number of carbons n is at least 6.

The number of carbons n is more preferably at least 12 when viewed from the standpoint of the affinity with the carrier liquid. The upper limit on the number of carbons n is preferably not more than 30 and is more preferably not more than 22. At least one hydrogen atom in the alkyl group, cycloalkyl group, alkylene group, or cycloalkylene group may be substituted.

The substituent that may be present on the alkyl group, cycloalkyl group, alkylene group, or cycloalkylene group encompassed by Q is not particularly limited and can be exemplified by alkyl groups, alkoxy groups, halogen atoms, the amino group, the hydroxy group, the carboxy group, carboxylate ester groups, and carboxamide groups.

The monomer unit represented by formula (1) is more preferably the monomer unit represented by the following formula (3).



[In formula (3), A represents a single bond, an alkylene group having 1 to 6 carbons (preferably 1 to 3 carbons), or a phenylene, and m represents an integer from 0 to 3.]

The monomer unit represented by formula (1) is still more preferably the monomer unit represented by the following formula (4).



On the other hand, the monomer unit represented by formula (2) is more preferably the monomer unit represented by the following formula (5).



[In formula (5), R<sub>1</sub> represents a possibly substituted alkyl group having at least 6 carbons or a possibly substituted cycloalkyl group having at least 6 carbons, and L represents a divalent linker group.]

R<sub>1</sub> is represented by the straight-chain  $—C_nH_{2n+1}$  or cyclic  $—C_nH_{2n-1}$  and denotes an alkyl group or cycloalkyl group in which n is at least 6.

n is more preferably at least 12. The upper limit for n, on the other hand, is preferably not more than 30 and is more preferably not more than 22.

In addition, the substituent that may be present on R<sub>1</sub> is not particularly limited and can be exemplified by alkyl groups, alkoxy groups, halogen atoms, the amino group, the hydroxy group, the carboxy group, carboxylate ester groups, and carboxamide groups.

L represents a divalent linker group and is preferably an alkylene group having 1 to 6 carbons (more preferably an alkylene group having 1 to 3 carbons), an alkenylene group having 1 to 6 carbons (more preferably an alkenylene group having 1 to 3 carbons), or an arylene group having 6 to 10 carbons.

In another more preferred embodiment, the monomer unit represented by formula (2) is the monomer unit represented by the following formula (6).



The R<sub>2</sub> in formula (6) is a possibly substituted alkylene group having at least 6 carbons or a possibly substituted cycloalkylene group having at least 6 carbons. p represents an integer with a value of at least 1 (preferably from 2 to 20). L represents a divalent linker group.

R<sub>2</sub> is represented by the straight-chain  $—C_nH_{2n—}$  or cyclic  $—C_nH_{2n-2—}$  and denotes an alkylene group or cycloalkylene group having at least 6 carbons. The number of carbons in the alkylene group or cycloalkylene group is more preferably at least 12. The upper limit for the number of carbons, on the other hand, is preferably not more than 30 and is more preferably not more than 22.

In addition, the substituent that may be present on R<sub>2</sub> is not particularly limited and can be exemplified by alkyl groups, alkoxy groups, halogen atoms, the amino group, the hydroxyl group, the carboxy group, carboxylate ester groups, and carboxamide groups.

Preferred examples for L are the same as for formula (5). The monomer unit represented by formula (1) may be a combination of any such monomer units, and the monomer unit represented by formula (2) may be a combination of any such monomer units.

The primary amino group-bearing polymer is preferably a polyallylamine derivative that contains the monomer unit represented by formula (4) in the polymer.

The number of monomer units represented by formula (4) present in each molecule of this polyallylamine derivative is preferably, as an average, from 10 to 200, more preferably from 20 to 150, and still more preferably from 50 to 150.

In addition, this primary amino group-bearing polymer is more preferably a polyallylamine derivative that contains, in one and the same polymer, the monomer unit represented by formula (4) and the monomer unit represented by formula (6).

The molar ratio between the monomer unit with formula (4) and the monomer unit with formula (6) [monomer unit

## 11

with formula (4): monomer unit with formula (6)] in this polymer is preferably 10:90 to 90:10 and is more preferably 50:50 to 80:20.

The polyallylamine derivative is also more preferably a polyallylamine derivative as provided by the reaction of a polyallylamine with the self-condensate of 12-hydroxystearic acid. Such a polyallylamine derivative can be synthesized by the method disclosed in, for example, Japanese Patent No. 3,718,915.

In addition, a commercially available polyamine compound and polyamine compound solution may be used to produce this polyallylamine derivative. Examples here are PAA-01, PAA-1LV, PAA-03, PAA-05, PAA-08, PAA-15, PAA-15C, PAA-25, and PAA-03E (Nittobo Medical Co., Ltd).

The amine value of the toner particle dispersing agent is at least 40 mg KOH/g. When the amine value is made at least 40 mg KOH/g, adsorption with the acid groups of the polyester resin A present at the toner particle surface can occur at multiple points, which supports strong retention by the toner particle and increases the dispersion stability.

The amine value is preferably at least 60 mg KOH/g. When the amine value is made at least 60 mg KOH/g, adsorption with the acid groups of the polyester resin A present at the toner particle surface can be realized at even more points, which supports an even greater increase in the dispersion stability.

The upper limit on the amine value is not particularly limited, but is generally not more than 300 mg KOH/g and is preferably not more than 200 mg KOH/g.

Moreover, it was found that a liquid developer having a high dispersion stability can be produced by having the SP value of the polyester resin B and the SP value of the liquid a satisfy the following formula (7).

$$SP_{carrier} < \left( \frac{E_d + a \times n \times E_p}{(V_d + a \times n \times V_p)} \right)^{0.5} < SP_{PESB} \quad (7)$$

[In formula (7), Ed and Ep respectively represent the cohesive energy of the toner particle dispersing agent and the polyester resin A, and Vd and Vp respectively represent the molar volume of the toner particle dispersing agent and the polyester resin A. Also, a represents the number-average number of amino groups per molecule with respect to the average degree of polymerization of the toner particle dispersing agent, and n represents the number-average degree of polymerization of the polyester resin A. SP<sub>Carrier</sub> represents the SP value of the liquid a, and SP<sub>PESB</sub> represents the SP value of the polyester resin B.]

The SP value is the solubility parameter. The SP value is a value introduced by Hildebrand and defined by a formal theory, and it is given by the square root of the cohesive energy density of the solvent (or solute) and is a measure of the solubility in a two-component system solution.

The SP value, cohesive energy, and molar volume of the liquid a, polyester resin A, polyester resin B, and toner particle dispersing agent are the values determined by calculation from the vaporization energy and molar volume of the atoms and atomic groups in accordance with Fedors as described in Coating Basics and Engineering (page 53, Yuji Harasaki, Converting Technical Institute).

The unit for the SP value in the present invention is (cal/cm<sup>3</sup>)<sup>1/2</sup>, but this can be converted to the (J/m<sup>3</sup>)<sup>1/2</sup> unit using 1 (cal/cm<sup>3</sup>)<sup>1/2</sup>=2.046×10<sup>3</sup> (J/m<sup>3</sup>)<sup>1/2</sup>.

## 12

The second term in formula (7) is a value that resembles the SP value of the polyester resin A-bonded toner particle dispersing agent. When formula (7) is satisfied, a force positioned between that for the liquid a and the polyester resin B acts for the polyester resin A-bonded toner particle dispersing agent. It is thought that this facilitates the presence of the polyester resin A-bonded toner particle dispersing agent at the interface between the toner particle and the liquid a and that the effects of the present invention are then even more substantially expressed.

## Liquid Developer

In addition to the insulating liquid carrier, the toner particle dispersing agent, and the toner particle containing the polyester resin A and the polyester resin B, the liquid developer may as necessary contain a colorant, charge control agent, charge adjuvant, and other additives, as described below.

When the insulating liquid carrier of the liquid developer is a cationically polymerizable liquid monomer, a photopolymerization initiator, sensitizer, cationic polymerization inhibitor, and other additives may also be incorporated.

## Insulating Liquid Carrier

The insulating liquid carrier exhibits an electrical insulating behavior and preferably has a volume resistivity of 1×10<sup>9</sup> to 1×10<sup>13</sup> Ω·cm. For example, it can be selected from the same materials as for the liquid a. Preferably liquid a is an insulating liquid carrier.

In specific terms, cationically polymerizable liquid monomers, e.g., vinyl ether compounds, and Moresco White MT-30P and so forth are preferred. Vinyl ether compounds are more preferred.

With regard to the insulating liquid carrier, when the liquid a used in the process A is of the appropriate type, it may be used as such as the carrier liquid of the liquid developer, or it may be replaced by a desired insulating liquid carrier by, for example, decantation or filtration. Considered from a productivity standpoint, in a more preferred embodiment an insulating liquid carrier is preliminarily used as the liquid a and is then used as such.

## Colorant

The toner particle in the present invention may contain a colorant. There are no particular limitations on this colorant, and, for example, the following can be used: any generally commercially available organic pigment, organic dye, or inorganic pigment; a pigment dispersed in, for example, an insoluble resin as the dispersion medium; or a colorant provided by grafting a resin onto the surface of a pigment.

The following are specific examples of pigments that exhibit a yellow color:

C. I. Pigment Yellow 1, 2, 3, 4, 5, 6, 7, 10, 11, 12, 13, 14, 15, 16, 17, 23, 62, 65, 73, 74, 83, 93, 94, 95, 97, 109, 110, 111, 120, 127, 128, 129, 147, 151, 154, 155, 168, 174, 175, 176, 180, 181, and 185, and C. I. Vat Yellow 1, 3, and 20.

The following are examples of pigments that exhibit a red or magenta color:

C. I. Pigment Red 1, 2, 3, 4, 5, 6, 7, 8, 9, 10, 11, 12, 13, 14, 15, 16, 17, 18, 19, 21, 22, 23, 30, 31, 32, 37, 38, 39, 40, 41, 48:2, 48:3, 48:4, 49, 50, 51, 52, 53, 54, 55, 57:1, 58, 60, 63, 64, 68, 81:1, 83, 87, 88, 89, 90, 112, 114, 122, 123, 146, 147, 150, 163, 184, 202, 206, 207, 209, 238, and 269; C. I. Pigment Violet 19; and C. I. Vat Red 1, 2, 10, 13, 15, 23, 29, and 35.

The following are examples of pigments that exhibit a blue or cyan color:

C. I. Pigment Blue 2, 3, 15:2, 15:3, 15:4, 16, and 17; C. I. Vat Blue 6; C. I. Acid Blue 45; and copper phthalocyanine

13

pigments in which 1 to 5 phthalimidomethyl groups are substituted on the phthalocyanine skeleton.

The following are examples of pigments that exhibit a green color:

C. I. Pigment Green 7, 8, and 36.

The following are examples of pigments that exhibit an orange color:

C. I. Pigment Orange 66 and 51.

The following are examples of pigments that exhibit a black color:

carbon black, titanium black, and aniline black.

The following are examples of pigments that exhibit a white color:

basic lead carbonate, zinc oxide, titanium oxide, and strontium titanate.

The content of the colorant, per 100 mass parts of the binder resin, is preferably 1 to 100 mass parts and more preferably 5 to 50 mass parts.

A dispersing means adapted to the toner particle production method should be used to disperse the pigment in the toner particle. Examples of devices that can be used as the dispersing means are ball mill, sand mill, attritor, roll mill, jet mill, homogenizer, paint shaker, kneader, agitator, Henschel mixer, colloid mill, ultrasound homogenizer, pearl mill, and wet jet mill.

A pigment dispersing agent may also be added during pigment dispersion. This pigment dispersing agent can be exemplified by hydroxyl group-containing carboxylate esters, salts between long-chain polyaminoamides and high molecular weight acid esters, salts of high molecular weight polycarboxylic acids, high molecular weight unsaturated acid esters, high molecular weight copolymers, modified polyacrylates, polybasic aliphatic carboxylic acids, naphthalenesulfonic acid/formalin condensates, polyoxyethylene alkyl phosphate esters, and pigment derivatives. The use of commercial high molecular weight dispersing agents, e.g., the Solperse series (Lubrizol Japan Ltd.), is also preferred.

A synergist corresponding to various pigments may also be used as a pigment dispersion auxiliary. The amount of addition of these pigment dispersing agents and pigment dispersion auxiliaries is preferably from 1 mass parts to 50 mass parts per 100 mass parts of the pigment.

Charge Control Agent

The liquid developer may optionally contain a charge control agent. A known charge control agent may be used here.

The following are examples of specific compounds:

fats and oils such as linseed oil and soybean oil; alkyd resins; halogen polymers; aromatic polycarboxylic acids; acidic group-containing water-soluble dyes; oxidative condensates of aromatic polyamines; metal soaps such as cobalt naphthenate, nickel naphthenate, iron naphthenate, zinc naphthenate, cobalt octylate, nickel octylate, zinc octylate, cobalt dodecylate, nickel dodecylate, zinc dodecylate, aluminum stearate, and cobalt 2-ethylhexanoate; sulfonate metal salts such as petroleum metal sulfonates and metal salts of sulfosuccinate esters; phospholipids such as hydrogenated lecithin and lecithin; metal salicylate salts such as metal complexes of t-butylsalicylic acid; as well as polyvinylpyrrolidone resins, polyamide resins, sulfonic acid-containing resins, and hydroxybenzoic acid derivatives.

The charge control agent optionally added to the liquid developer can be added after toner particle production. In the case of wet pulverization, it can be added during wet pulverization and/or after wet pulverization.

14

Charge Adjuvant

The toner particle may contain a charge adjuvant with the goal of adjusting the charging performance of the toner particle. A known charge adjuvant can be used as this charge adjuvant.

The following are examples of specific compounds: metal soaps such as zirconium naphthenate, cobalt naphthenate, nickel naphthenate, iron naphthenate, zinc naphthenate, cobalt octylate, nickel octylate, zinc octylate, cobalt dodecylate, nickel dodecylate, zinc dodecylate, aluminum stearate, aluminum tristearate, and cobalt 2-ethylhexanoate; sulfonate metal salts such as petroleum metal sulfonates and metal salts of sulfosuccinate esters; phospholipids such as hydrogenated lecithin and lecithin; metal salicylate salts such as metal complexes of t-butylsalicylic acid; as well as polyvinylpyrrolidone resins, polyamide resins, sulfonic acid-containing resins, and hydroxybenzoic acid derivatives.

Other Additives

Besides the preceding, various known additives may be used on an optional basis in the liquid developer with the goals of improving the recording medium compatibility, storage stability, image storability, and other properties. For example, the following can be selected as appropriate and used: surfactants, lubricants, fillers, defoamants, ultraviolet absorbers, oxidation inhibitors, antifading agents, antimolds, rust inhibitors, and so forth.

Photopolymerization Initiator

The photopolymerization initiator is a compound that reacts to light at a designated wavelength and thereby generates an acid or a radical. Within the sphere of such compounds, cationic photopolymerization initiators can be exemplified by onium salt compounds, sulfone compounds, sulfonate ester compounds, sulfonimide compounds, and diazomethane compounds, but are not limited to these.

Moreover, when a cationic photopolymerization initiator is used in the present invention, the use is more preferred of a photopolymerization initiator represented by the following formula (8), which causes little reduction in the volume resistivity of ultraviolet curable liquids.



[In formula (8), R<sub>1</sub> and R<sub>2</sub> are bonded to each other to form a ring structure; x represents an integer from 1 to 8; and y represents an integer from 3 to 17.]

The ring structure formed by the bonding of R<sub>1</sub> with R<sub>2</sub> can be exemplified by 5-membered rings and 6-membered rings. These ring structures may also have the following as substituents: an alkyl group, an alkoxy group, an alkylthio group, an aryl group, and an aryloxy group. Moreover, other, possibly substituted cyclic structures, e.g., alicyclic rings, heterocyclic rings, aromatic rings, and so forth, may also be condensed. Examples of preferred ring structures are succinimide structures, phthalimide structures, norbornene dicarboximide structures, naphthalene dicarboximide structures, cyclohexane dicarboximide structures, and epoxycyclohexene dicarboximide structures.

The C<sub>x</sub>F<sub>y</sub> in general formula (8) can be exemplified by straight-chain alkyl groups in which the hydrogen atom has been substituted by the fluorine atom (RF<sub>1</sub>), branched-chain

## 15

alkyl groups in which the hydrogen atom has been substituted by the fluorine atom (RF2), cycloalkyl groups in which the hydrogen atom has been substituted by the fluorine atom (RF3), and aryl groups in which the hydrogen atom has been substituted by the fluorine atom (RF4).

The straight-chain alkyl groups in which the hydrogen atom has been substituted by the fluorine atom (RF1) can be exemplified by the trifluoromethyl group (x=1, y=3), pentafluoroethyl group (x=2, y=5), nonafluorobutyl group (x=4, y=9), perfluorohexyl group (x=6, y=13), and perfluoroctyl group (x=8, y=17).

The branched-chain alkyl groups in which the hydrogen atom has been substituted by the fluorine atom (RF2) can be exemplified by the perfluoroisopropyl group (x=3, y=7), perfluoro-tert-butyl group (x=4, y=9), and perfluoro-2-ethylhexyl group (x=8, y=17).

The cycloalkyl groups in which the hydrogen atom has been substituted by the fluorine atom (RF3) can be exemplified by the perfluorocyclobutyl group (x=4, y=7), perfluorocyclopentyl group (x=5, y=9), perfluorocyclohexyl group (x=6, y=11), and perfluoro (1-cyclohexyl) methyl group (x=7, y=13).

The aryl groups in which the hydrogen atom has been substituted by the fluorine atom (RF4) can be exemplified by the pentafluorophenyl group (x=6, y=5) and 3-trifluoromethyltetrafluorophenyl group (x=7, y=7).

For the  $C_xF_y$  in general formula (8), the straight-chain alkyl groups (RF1), branched-chain alkyl groups (RF2), and aryl groups (RF4) are preferred from the standpoint of the ease of acquisition and the decomposability of the sulfonate ester moiety. The straight-chain alkyl groups (RF1) and aryl groups (RF4) are more preferred, while the trifluoromethyl group (x=1, y=3), pentafluoroethyl group (x=2, y=5), heptafluoropropyl group (x=3, y=7), nonafluorobutyl group (x=4, y=9), and pentafluorophenyl group (x=6, y=5) are particularly preferred.

A single photopolymerization initiator can be used or two or more can be used in combination. The content of the photopolymerization initiator in the liquid developer is not particularly limited, but, expressed per 100 mass parts of the cationically polymerizable liquid monomer, is preferably from 0.01 mass parts to 5 mass parts, more preferably from 0.05 mass parts to 1 mass parts, and even more preferably from 0.1 mass parts to 0.5 mass parts.

Specific examples of the photopolymerization initiator with formula (8) [exemplary compounds A-1 to A-27] are provided below, but the present invention is not limited to or by these examples.

## 16

-continued

(A-3)



(A-4)



(A-5)



(A-6)



(A-7)



(A-8)



(A-9)



(A-10)



65



**17**  
-continued

(A-11)



5

(A-12)



10

(A-13)



15

(A-14)



20

(A-15)



25

(A-16)



30

(A-17)



35

(A-18)



40

(A-19)

**18**  
-continued

(A-19)



(A-20)



(A-21)



(A-22)



(A-23)



(A-24)



(A-25)



(A-26)



19

-continued

(A-27)



## Additives

Additives such as the following are preferably incorporated on an optional basis when the liquid developer is made into a cationically polymerizable, ultraviolet-curable liquid developer.

## Sensitizer

A sensitizer may be added on an optional basis to the cationically polymerizable, ultraviolet-curable liquid developer with the goals of improving the acid-generating efficiency of the photo-acid generator, extending the photosensitive wavelengths to longer wavelengths, and so forth. Any sensitizer may be used that is capable of sensitizing the photopolymerization initiator through an electron transfer mechanism or energy transfer mechanism.

Preferred examples are aromatic polycondensed ring compounds such as anthracene, 9,10-dialkoxyanthracene, pyrene, and perylene; aromatic ketone compounds such as acetophenone, benzophenone, thioxanthone, and Michler's ketone; and heterocyclic compounds such as phenothiazine and N-aryloxazolidinone. The amount of addition is selected as appropriate in correspondence to the goal, and generally preferably from 0.1 mass parts to 10 mass parts and more preferably from 1 mass parts to 5 mass parts is used per 1 mass parts of the polymerization initiator.

In a preferred embodiment, a co-sensitizer is also added to the cationically polymerizable, ultraviolet-curable liquid developer with the goal of improving the electron transfer efficiency or energy transfer efficiency between the aforementioned sensitizer and the photopolymerization initiator. The co-sensitizer can be specifically exemplified by the following: naphthalene compounds such as 1,4-dihydroxynaphthalene, 1,4-dimethoxynaphthalene, 1,4-diethoxynaphthalene, 4-methoxy-1-naphthol, and 4-ethoxy-1-naphthol, and benzene compounds such as 1,4-dihydroxybenzene, 1,4-dimethoxybenzene, 1,4-diethoxybenzene, 1-methoxy-4-phenol, and 1-ethoxy-4-phenol.

The amount of co-sensitizer addition is selected as appropriate in correspondence to the goal, but is, per 1 mass parts of the sensitizer, preferably from 0.1 mass parts to 10 mass parts and more preferably from 0.5 mass parts to 5 mass parts.

## Cationic Polymerization Inhibitor

A cationic polymerization inhibitor may also be added to the cationically polymerizable, ultraviolet-curable liquid developer. The cationic polymerization inhibitor can be exemplified by alkali metal compounds and/or alkaline-earth metal compounds and by amines.

Alkanolamines, N,N-dimethylalkylamines, N,N-dimethylalkenylamines, and N,N-dimethylalkynylamines are preferred for the amines and can be specifically exemplified by triethanolamine, triisopropanolamine, tributanolamine, N-ethyldiethanolamine, propanolamine, n-butylamine, sec-butylamine, 2-aminoethanol, 2-methylaminoethanol, 3-methylamino-1-propanol, 3-methylamino-1,2-propanediol, 2-ethylaminoethanol, 4-ethylamino-1-butanol, 4-(n-butylamino)-1-butanol, 2-(t-butylamino)ethanol, N,N-dim-

20

ethylundecanolamine, N,N-dimethyldodecanolamine, N,N-dimethyltridecanolamine, N,N-dimethyltetradecanolamine, N,N-dimethylpentadecanolamine, N,N-dimethylnonadecylamine, N,N-dimethyllicosylamine, N,N-dimethyleicosylamine, N,N-dimethylheneicosylamine, N,N-dimethyldecosylamine, N,N-dimethyltricosylamine, N,N-dimethylpentacosylamine, N,N-dimethylhexanolamine, N,N-dimethylheptanolamine, N,N-dimethyloctanolamine, N,N-dimethylnonanolamine, N,N-dimethyldecanolamine, N,N-dimethylnonylamine, N,N-dimethyldecylamine, N,N-dimethylundecylamine, N,N-dimethyldodecylamine, N,N-dimethyltridecylamine, N,N-dimethyltetradecylamine, N,N-dimethylpentadecylamine, N,N-dimethylhexadecylamine, N,N-dimethylheptadecylamine, and N,N-dimethyloctadecylamine. In addition to these, for example, a quaternary ammonium salt may also be used. The cationic polymerization inhibitor is particularly preferably a secondary amine.

The amount of addition of the cationic polymerization inhibitor is preferably from 10 ppm to 5,000 ppm on a mass basis in the ultraviolet-curable liquid developer.

## Toner Particle Production Process A

The toner particle production process A is described in detail in the following. The process A in the present invention has

a step of particulating a mixture of the polyester resin A, the polyester resin B, and the toner particle dispersing agent in a liquid a by applying shear force to the mixture, and

a step of producing a toner particle in the liquid a via a molten state.

For example, in a general method, heating and kneading are carried out using, e.g., a three-roll mill, twin-screw extruder, and so forth, at a temperature higher than the softening points of both resins, i.e., the polyester resin A and the polyester resin B, followed by a dry pulverization using a pulverizer, e.g., a hammer mill, jet mill, pin mill, turbo mill, cutter mill, ball mill, and so forth, to obtain a finely particulated material.

The liquid a and the toner particle dispersing agent are then added to this finely particulate material and a wet pulverization is subsequently performed using a wet pulverizer such as a media-based disperser, e.g., an attritor, sand mill, Dyno mill, ball mill, DCP mill, Apex mill, pearl mill, and so forth, or such as a media-free pulverizer, e.g., an Ultimizer (Sugino Machine Limited), Nanomizer (Nanomizer Inc.), and so forth. By doing this, shear force is applied to the mixture and particulation can be brought about and a suspension containing toner particles in the liquid a can be produced. There is no particular limitation on the applied shear force, and it should be selected as appropriate in conformity with the desired particle diameter.

By proceeding through a molten state in the liquid a, and in accordance with the specified sequence for the SP values, the polyester resin B moves into the interior of the toner particle; orientation of the toner particle dispersing agent and polyester resin A, while they are in a state of adsorptive interaction, to the toner particle surface is facilitated; and a toner having an excellent dispersion stability can be produced.

In order to establish a molten state, for example, as a general method it is sufficient to establish a temperature higher than the softening points of both resins, i.e., the polyester resin A and the polyester resin B. For example, a hot plate, oil bath, oven, thermostat, and so forth, may be used without particular limitation. The temperature conditions are, for example, heating for preferably 10 minutes to 1,440 minutes and more preferably for 20 minutes to 360

## 21

minutes, at preferably 60° C. to 200° C. and more preferably 80° C. to 150° C. In addition, coarsening of the pulverized particles can be prevented during the melt interval by, as necessary, causing the suspension to undergo a gentle flow using, for example, a stirring bar, stirring blade, mixing rotor, shaker, and so forth.

## Toner Particle Production Process B

The toner particle production process B is described in detail in the following.

The process B in the present invention has

a step of dissolving, in a solvent b, a mixture of the polyester resin A, the polyester resin B, and the toner particle dispersing agent;

a step of mixing the resulting solution with the liquid a and applying shear force to particulate the mixture in the liquid a and provide a toner particle; and

a step of distillatively removing the solvent b.

As a general method, for example, the toner particle may also be produced by the coacervation method.

First, using a solvent b that dissolves the polyester resin

A, the polyester resin B, and the toner particle dispersing agent, their mixture is dissolved therein with thorough stirring. Then, while adding the liquid a, the mixture is particulated by applying a shear force to produce a suspension that contains the toner particle in the liquid a and solvent b.

The shear force may be set as appropriate in conformity with the desired particle diameter. With regard to high-velocity shearing apparatuses capable of applying a high shear force, dispersers that operate by high-speed stirring, e.g., homogenizers, homomixers, and so forth, which apply a stirring shear, can uniformly apply a high shear force to the toner particle and are thus preferred. With regard to capacity, rotation rate, configuration, and so forth, various such apparatuses are available, and the appropriate apparatus should be selected in conformity with the production mode.

The rotation rate in the case of use of a homogenizer is preferably from 500 rpm to 30,000 rpm and is more preferably from 13,000 rpm to 28,000 rpm. The temperature in the mixing step is preferably at least the freezing points and not more than the boiling points of the solvent b and liquid a. The range from 0° C. to 60° C. is specifically preferred.

The step of distillatively removing the solvent b is then carried out. The solvent b is distillatively removed from the suspension containing toner particles in the liquid a and solvent b. For example, a method such as evaporation is suitable for the distillative removal method. For the conditions, distillative removal at 0° C. to 60° C. under reduced pressure at a pressure of 1 to 200 kPa is preferred. The execution of the distillative removal step produces a suspension containing toner particles in the liquid a.

## Liquid Developer Production Process

The liquid developer production process is described in detail in the following.

With regard to the suspension containing toner particles in the liquid a, as produced in the toner particle production process A, the liquid a can be used as such as long as this poses no problems with respect to the properties of the liquid developer, e.g., resistance, volatility, and so forth. While substitution may as necessary be carried out by a method such as filtration or decantation to an insulating liquid carrier c suitable as a carrier for liquid developers, the use of liquid a as such is desirable from the standpoint of mass productivity.

## Solvent b

A solvent can be used when the toner particle is produced by the coacervation method. The solvent b preferably can

## 22

dissolve the polyester resin A, the polyester resin B, and the toner particle dispersing agent. Examples here are ethers such as tetrahydrofuran, ketones such as methyl ethyl ketone and cyclohexanone, esters such as ethyl acetate, and halogenated compounds such as chloroform. This may also be an aromatic hydrocarbon capable of dissolving the resins, e.g., toluene, benzene, and so forth.

## Image-Forming Apparatus

The liquid developer can be advantageously used in ordinary or common image-forming apparatuses that employ an electrophotographic system.

## EXAMPLES

The present invention is described in detail in the following using examples, but the present invention is not limited to or by these examples. Unless specifically indicated otherwise, "parts" and "%" denote, respectively, "mass parts" and "mass %".

## Measurement Methods

The measurement methods using in the examples are described in the following. (1) Method for Measuring Molecular Weight [Weight-average Molecular Weight (Mw) and Number-average Molecular Weight (Mn)]

The molecular weight of, e.g., the resins, was determined on a polystyrene basis using gel permeation chromatography (GPC). The measurement of molecular weight by GPC was carried out as described in the following.

Sample sufficient to provide a sample concentration of 1.0 mass % was added to the eluent indicated below, and a solution in which the sample was dissolved was prepared by standing for 24 hours at room temperature. This solution was filtered across a solvent-resistant membrane filter having a pore diameter of 0.20  $\mu$ m to provide the sample solution, and the measurement was run using the following conditions.

Instrument: "HLC-8220GPC" high-performance GPC instrument [Tosoh Corporation]

Column: 2xLF-804

Eluent: tetrahydrofuran (THF)

Flow rate: 1.0 mL/min

Oven temperature: 40° C.

Sample injection amount: 0.025 mL

A molecular weight calibration curve constructed using polystyrene resin standards [Tosoh Corporation, TSK Standard Polystyrene F-850, F-450, F-288, F-128, F-80, F-40, F-20, F-10, F-4, F-2, F-1, A-5000, A-2500, A-1000, A-500] was used to determine the molecular weight of the sample.

## (2) Method for Measuring Acid Value

The acid value of the resins is determined using the following method.

The basic procedure is based on JIS K 0070.

1) 0.5 to 2.0 g of the sample is exactly weighed. This mass is designated M1 (g).

2) The sample is introduced into a 50-mL beaker. 25 mL of a tetrahydrofuran/ethanol mixed solvent (2/1) is added and dissolution is carried out.

3) Titration is performed using a 0.1 mol/L ethanolic KOH solution and a potentiometric titrator [a "COM-2500" Automatic Titrator from Hiranuma Sangyo Co., Ltd. can be used].

4) The amount of the KOH solution used here is designated A (mL). The blank is measured at the same time, and the amount of KOH used in this case is designated B (mL).

5) The acid value is calculated using the following formula (i). Here, f refers to the factor for the KOH solution.

$$\text{Acid Value [mg KOH/g]} = \frac{[(A + B) \times f \times 5.61]}{M} \quad (i)$$

### (3) Methods for Measuring Amine Value

The amine value of the resins and the toner particle dispersing agents is determined using the following method.

The basic procedure is based on ASTM D 2074.

1) 0.5 to 2.0 g of the sample is exactly weighed. This mass is designated M (g).

2) The sample is introduced into a 50-mL beaker. 25 mL of tetrahydrofuran/ethanol mixed solvent (3/1) is added and dissolution is carried out.

3) Titration is performed using a 0.1 mol/L ethanolic HCl solution and a potentiometric titrator [a "COM-2500" Automatic Titrator from Hiranuma Sangyo Co., Ltd. can be used].

4) The amount of the HCl solution used here is designated S (mL). The blank is measured at the same time, and the amount of HCl used in this case is designated B (mL).

5) The amine value is calculated using the following formula. Here, f is the factor for the HCl solution.

$$\text{Amine Value [mg KOH/g]} = \frac{(S - B) \times f \times 5.61}{M} \quad (ii)$$

### Measurement of Acid Value of Toner Particle and Amine Value of Toner Dispersing Agent from Liquid Developer

The following method is used to determine the acid value of the binder resin and the amine value of the toner dispersing agent contained in the toner particle in the ultraviolet-curable liquid developer.

1) Approximately 10 g of the ultraviolet-curable liquid developer is subjected to centrifugal separation: the toner particles are sedimented and the supernatant is discarded.

2) Hexane is then added to the toner particles with thorough stirring followed by centrifugal separation: the toner particles are sedimented and the supernatant is discarded. This sequence is carried out three times followed by thorough drying.

3) 10 g of tetrahydrofuran is added to 2) and standing overnight is carried out. After thorough stirring, this is then subjected to centrifugal separation and the tetrahydrofuran-insoluble component is removed. The tetrahydrofuran-soluble component (binder resin and toner particle dispersing agent mixture) in the supernatant is thoroughly dried.

4) Using the methods described above, the acid value and amine value are measured on the tetrahydrofuran-soluble component obtained in 3).

In addition, as necessary:

(i) the toner particle obtained in 2) above is dissolved in deuteriochloroform and the primary amino group-bearing polymer and the polyester resin constituting the toner particle are subjected to compositional analysis using a JNM-ECA (<sup>1</sup>H-NMR) Fourier-transform nuclear magnetic resonance instrument from JEOL Ltd.;

(ii) on the other hand, the number-average molecular weight (Mn) of the tetrahydrofuran-soluble component

obtained in 3) above is determined using gel permeation chromatography (GPC), and the number-average degree of polymerization of the polyester resin and the average degree of polymerization of the primary amino group-bearing polymer are determined from the results in (i) and (ii).

### Polyester Resin A Production Examples

#### Polyester PESA-1 Production Example

10 The following were introduced into a reaction kettle equipped with a stirrer, thermometer, and reflux condenser and subjected to an esterification reaction for 2 hours at 220° C.: 82 parts of terephthalic acid, 82 parts of isophthalic acid, 212 parts of the 2 mol adduct of ethylene oxide on bisphenol A, 48 parts of ethylene glycol, 31 parts of neopentyl glycol, 0.1 parts of n-tetrabutyl titanate as catalyst, 2 parts of Irganox 1330 (BASF Japan Ltd.) as antioxidant, and 0.3 parts of sodium acetate as polymerization stabilizer.

20 The pressure within the system was then reduced while raising the temperature of the reaction system from 220° C. to 270° C., and a polycondensation reaction was subsequently run for 10 minutes at or below 1 Torr. After 25 completion of the reaction, the system was returned from the vacuum to normal pressure using nitrogen. 21 parts of trimellitic anhydride was introduced as the polycarboxylic acid that would provide the acid value, and a reaction was run for 30 minutes at 220° C. to obtain a polyester.

30 100 parts of the obtained polyester was dissolved in 200 parts of chloroform; this was introduced along with 300 parts of deionized water into a separatory funnel; agitation and standing at quiescence were performed; and the upper layer was discarded. The lower layer was washed twice with water followed by distillative removal of the chloroform using an evaporator to obtain the polyester PESA-1.

#### Polyester Resin A PESA-2 Production Example

35 The following were introduced into a reaction kettle equipped with a stirrer, thermometer, and reflux condenser and subjected to an esterification reaction for 2 hours at 220° C.: 82 parts of terephthalic acid, 82 parts of isophthalic acid, 14 parts of trimellitic anhydride, 212 parts of the 2 mol adduct of ethylene oxide on bisphenol A, 48 parts of ethylene glycol, 31 parts of neopentyl glycol, 0.1 parts of n-tetrabutyl titanate as catalyst, 2 parts of Irganox 1330 as 45 antioxidant, and 0.3 parts of sodium acetate as polymerization stabilizer. The pressure within the system was then reduced while raising the temperature of the reaction system from 220° C. to 270° C., and a polycondensation reaction 50 was subsequently run for 11 minutes at or below 1 Torr. After completion of the reaction, the system was returned from the vacuum to normal pressure using nitrogen to yield the polyester PESA-2.

#### Polyester Resins A PESA-3 to PESA-5 and Polyester Resins A PESA-101 to PESA-104 Production Examples

55 Polyester resins A PESA-3 to PESA-5 and polyester resins A PESA-101 to PESA-104 were obtained by the same reaction, but changing the method described in the example 60 for the synthesis of polyester PESA-2 to the method described in Table 1.

TABLE 1

| BPA-EO   | EG  | NPG | TPA | IPA | TMA | Time of addition of trimellitic anhydride | Polycondensation reaction time [min] |    |
|----------|-----|-----|-----|-----|-----|-------------------------------------------|--------------------------------------|----|
| PESA-1   | 212 | 48  | 31  | 82  | 82  | 21                                        | After polycondensation               | 10 |
| PESA-2   | 212 | 48  | 31  | 82  | 82  | 14                                        | Before polycondensation              | 11 |
| PESA-3   | 212 | 48  | 31  | 82  | 82  | 14                                        | Before polycondensation              | 7  |
| PESA-4   | 35  | 129 | 31  | 82  | 82  | 10                                        | Before polycondensation              | 19 |
| PESA-5   | 35  | 129 | 31  | 82  | 82  | 6                                         | Before polycondensation              | 20 |
| PESA-101 | 212 | 48  | 31  | 82  | 82  | 14                                        | Before polycondensation              | 27 |
| PESA-102 | 212 | 48  | 31  | 82  | 82  | 14                                        | Before polycondensation              | 3  |
| PESA-103 | 212 | 48  | 31  | 82  | 82  | 4                                         | Before polycondensation              | 10 |
| PESA-104 | 212 | 48  | 31  | 82  | 82  | 0                                         | No addition                          | 10 |

The numerical value for each monomer in the table indicates mass parts.

and subjected to an esterification reaction for 2 hours at 220° C.: 82 parts of terephthalic acid, 82 parts of isophthalic acid,

TABLE 2

| BPA-EO   | EG | NPG | TPA | IPA | TMA | Position of trimellitic anhydride |                   | Mn    | n    | SP value | Acid value |
|----------|----|-----|-----|-----|-----|-----------------------------------|-------------------|-------|------|----------|------------|
|          |    |     |     |     |     | 1                                 | Terminal position |       |      |          |            |
| PESA-1   | 6  | 3   | 1   | 5   | 5   | 1                                 | Terminal position | 4,100 | 9.8  | 11.8     | 14         |
| PESA-2   | 6  | 3   | 1   | 5   | 5   | 0.7                               | In main chain     | 4,200 | 10.0 | 11.8     | 10         |
| PESA-3   | 6  | 3   | 1   | 5   | 5   | 0.7                               | In main chain     | 3,100 | 7.4  | 11.8     | 10         |
| PESA-4   | 1  | 8   | 1   | 5   | 5   | 0.5                               | In main chain     | 6,800 | 24.0 | 12.5     | 10         |
| PESA-5   | 1  | 8   | 1   | 5   | 5   | 0.3                               | In main chain     | 6,900 | 24.3 | 12.4     | 5          |
| PESA-101 | 6  | 3   | 1   | 5   | 5   | 0.7                               | In main chain     | 9,000 | 21.4 | 11.8     | 10         |
| PESA-102 | 6  | 3   | 1   | 5   | 5   | 0.7                               | In main chain     | 2,000 | 4.8  | 11.8     | 10         |
| PESA-103 | 6  | 3   | 1   | 5   | 5   | 0.2                               | In main chain     | 4,000 | 9.5  | 11.7     | 3          |
| PESA-104 | 6  | 3   | 1   | 5   | 5   | 0                                 | No addition       | 4,100 | 9.8  | 11.7     | 1          |

In Table 2, the numerical values for each monomer in the obtained polyester are the results (molar ratio) from NMR measurement of the obtained polyester resin. The unit for the SP value is  $(\text{cal}/\text{cm}^3)^{1/2}$ , and the unit for the acid value is mg KOH/g. The abbreviations used in the tables and elsewhere have the following definitions.

BPA-EO: 2 mol ethylene oxide adduct on bisphenol A

EG: ethylene glycol

NPG: neopentyl glycol

TPA: terephthalic acid

IPA: isophthalic acid

TMA: trimellitic anhydride

Mn: number-average molec

n: number-average degree of polymerization

## Polyester Resin B (PESB-1) Production Example

The following were introduced into a reaction:

equipped with a stirrer, thermometer, and reflux condenser

5 parts of monosodium 5-sulfoisophthalate, 80 parts of ethylene glycol, 153 parts of neopentyl glycol, 0.1 parts of n-tetrabutyl titanate as catalyst, 2 parts of Irganox 1330 as antioxidant, and 0.3 parts of sodium acetate as polymerization stabilizer. The pressure within the system was then reduced while raising the temperature of the reaction system from 220° C. to 270° C., and a polycondensation reaction was subsequently run for 20 minutes at or below 1 Torr. After completion of the reaction, the system was returned from the vacuum to normal pressure using nitrogen to yield a polyester PESB-1.

## Polyester Resins B PESB-2 to PESB-5 and Polyester Resins B PESB-101 to PESB-103 Production Examples

Polyester resins B PESB-2 to PESB-5 and PESB-101 to PESB-103 were obtained by the same reaction, but changing the method described in the example for the synthesis of polyester PESB-1 to the method described in Table 3.

TABLE 3

|          | BPA-EO | EG | NPG | TPA | IPA | TMA | SIPA | Polycondensation    |                 |
|----------|--------|----|-----|-----|-----|-----|------|---------------------|-----------------|
|          |        |    |     |     |     |     |      | reaction time [min] | Acid value      |
| PESB-1   | 0      | 80 | 153 | 82  | 82  | 0   | 5    | 20                  | Not more than 2 |
| PESB-2   | 0      | 80 | 153 | 82  | 82  | 0   | 0    | 20                  | Not more than 2 |
| PESB-3   | 0      | 80 | 153 | 82  | 82  | 0   | 0    | 10                  | Not more than 2 |
| PESB-4   | 248    | 0  | 92  | 82  | 82  | 0   | 0    | 11                  | Not more than 2 |
| PESB-5   | 248    | 0  | 92  | 82  | 82  | 0   | 0    | 62                  | Not more than 2 |
| PESB-101 | 0      | 80 | 153 | 82  | 82  | 0   | 0    | 73                  | Not more than 2 |
| PESB-102 | 0      | 80 | 153 | 82  | 82  | 0   | 0    | 8                   | Not more than 2 |
| PESB-103 | 0      | 80 | 153 | 82  | 82  | 6   | 0    | 10                  | 5               |

The numerical value for each monomer in the table indicates mass parts.

TABLE 4

|          | BPA-EO | EG | NPG | TPA | IPA | TMA | SIPA | Mn     | SP value | Acid value      |
|----------|--------|----|-----|-----|-----|-----|------|--------|----------|-----------------|
| PESB-1   | 0      | 5  | 5   | 5   | 5   | 0   | 0.2  | 7,100  | 12.1     | Not more than 2 |
| PESB-2   | 0      | 5  | 5   | 5   | 5   | 0   | 0    | 7,100  | 12.0     | Not more than 2 |
| PESB-3   | 0      | 5  | 5   | 5   | 5   | 0   | 0    | 4,100  | 12.0     | Not more than 2 |
| PESB-4   | 7      | 0  | 3   | 5   | 5   | 0   | 0    | 4,200  | 11.4     | Not more than 2 |
| PESB-5   | 7      | 0  | 3   | 5   | 5   | 0   | 0    | 19,600 | 11.4     | Not more than 2 |
| PESB-101 | 0      | 5  | 5   | 5   | 5   | 0   | 0    | 23,000 | 12.0     | Not more than 2 |
| PESB-102 | 0      | 5  | 5   | 5   | 5   | 0   | 0    | 3,500  | 12.0     | Not more than 2 |
| PESB-103 | 0      | 5  | 5   | 5   | 5   | 0.3 | 0    | 4,000  | 12.1     | 5               |

15

In Table 4, the numerical values for each monomer in the obtained polyester are the results (molar ratio) from NMR measurement of the obtained polyester resin. The abbreviations are the same as those for Tables 1 and 2.

SIPA represents monosodium 5-sulfoisophthalate.

12-Hydroxystearic Acid Self-Condensate (P-1) Production Example

30.0 parts of xylene (Junsei Chemical Co., Ltd.), 300.0 parts of 12-hydroxystearic acid (Junsei Chemical Co., Ltd.), and 0.1 parts of tetrabutyl titanate (Tokyo Chemical Industry Co., Ltd.) were introduced into a reaction flask fitted with a thermometer, stirrer, nitrogen introduction line, reflux condenser, and water separator, and the temperature was raised over 4 hours to 160° C. under a nitrogen current. Heating was carried out for an additional 4 hours at 160° C. (the acid value at this point was approximately 20 mg KOH/g), and the xylene was distillatively removed at 160° C.

This was followed by cooling to room temperature; the water produced during the reaction under heating was separated from the xylene in the distillate; and this xylene was returned to the reaction solution. This reaction solution is designated below as 12-hydroxystearic acid self-condensate P-1. The polyester present in the 12-hydroxystearic acid self-condensate P-1 had the following properties: number-average molecular weight=2,550, acid value=22.0 mg KOH/g. Moreover, the thusly produced polyester can be used as a starting material for the synthesis of polyallylamine derivatives in a form associated with solvent (xylene).

Toner Particle Dispersing Agent Production Examples

Toner Particle Dispersing Agent Dis-1 Synthesis Example

A mixture of 25.0 parts of xylene and 70 parts of a 10% aqueous polyallylamine solution ("PAA-1LV", Nittobo Medical Co., Ltd., number-average molecular weight=approximately 3,000) was introduced into a reaction flask fitted with a thermometer, stirrer, nitrogen introduction line, and reflux condenser and heating was carried out to 160° C. while stirring. While distilling off the water using a separator and refluxing the xylene to the reaction solution, 12.8 parts of the 12-hydroxystearic acid self-condensate P-1 from the 12-Hydroxystearic Acid Self-Condensate (P-1) Production Example, heated to 160° C., was added thereto and a reaction was run at 160° C. for 2 hours to obtain a toner particle dispersing agent Dis-1 (amine value=60.0 mg KOH/g).

Toner Particle Dispersing Agents Dis-2 and Dis-101 Production Example

Toner particle dispersing agents Dis-2 and Dis-101 were obtained by the same reaction as in the Toner Particle

Dispersing Agent Dis-1 Synthesis Example, except for the amount of addition of the P-1.

TABLE 5

|    | polyallylamine | amount of P-1 addition | amine value of toner dispersing agent |
|----|----------------|------------------------|---------------------------------------|
| 20 | Dis-1          | PAA-1LV                | 12.8                                  |
|    | Dis-2          | PAA-1LV                | 13.8                                  |
|    | Dis-101        | PAA-1LV                | 14.8                                  |

Example of Liquid Developer Production by Wet Pulverization

#### Example 1

30 Liquid Developer Production Example (Process A)

21.6 parts of polyester resin A (PESA-1), 14.4 parts of polyester resin B (PESB-1), Pigment Blue 15:3 (9 parts), and 15 parts of Vylon UR4800 (Toyobo Co., Ltd., resin concentration=32%) were thoroughly mixed in a Henschel mixer and were then melt-kneaded using a co-rotating twin-screw extruder using a roll inner heating temperature of 100° C. The obtained mixture was cooled and coarsely pulverized to obtain a coarsely pulverized toner particle.

40 The following were then mixed for 48 hours using a sand mill: 160 parts Moresco White MT-30P (SP value=7.90) as liquid a, 40 parts of the coarsely pulverized toner particle obtained as described above, and 0.8 parts of the toner particle dispersing agent Dis-1. A toner particle dispersion T-1 was then obtained by stirring at 200 rpm under reflux while heating for 1 hour at 120° C. on an EC oil bath stirrer (AS ONE Corporation).

45 The liquid developer of Example 1 was obtained by mixing 0.10 parts of hydrogenated lecithin (Lecinol S-10, Nikko Chemicals Co., Ltd.) as a charge control agent into 10 parts of the obtained toner particle dispersion T-1.

#### Example 2

55 Liquid Developer Production Example (Process B)

Pigment Dispersion Production Step

Pigment Dispersion Production Example

55 Pigment Blue 15:3 (30 parts), Vylon UR4800 (47 parts), 255 parts of tetrahydrofuran, and 130 parts of glass beads (1 mm Ø) were mixed; dispersion was performed for 3 hours using an attritor [Nippon Coke & Engineering Co., Ltd.]; and filtration across a mesh was carried out to obtain a kneaded material.

60 180 parts of the obtained kneaded material, 69 parts of a 50% tetrahydrofuran solution of polyester resin A (PESA-1), 46 parts of a 50% tetrahydrofuran solution of polyester resin B (PESB-1), and 2.7 parts of the toner particle dispersing agent Dis-1 were mixed using a high-speed disperser (T. K.

Robomix/T. K. Homodisper Model 2.5 blade, PRIMIX Corporation) and were mixed while stirring at 40° C. to obtain a pigment dispersion.

#### Mixture Production Example

A mixture was obtained by adding 70 parts of Moresco White MT-30P as liquid a in small portions to 100 parts of the obtained pigment dispersion while stirring at high speed (25,000 rpm) using a homogenizer (Ultra-Turrax T50, IKA). Distillative Removal Step

The resulting mixture was transferred to a recovery flask and the tetrahydrofuran was completely distilled off at 50° C. while performing ultrasound dispersion to obtain a toner particle dispersion T-2.

#### Liquid Developer Preparation Step

The liquid developer of Example 2 was obtained by mixing 0.10 parts of hydrogenated lecithin (Lecinol S-10, Nikko Chemicals Co., Ltd.) as a charge control agent into 10 parts of the obtained toner particle dispersion T-2.

#### Example 3

##### Liquid Developer Production Example

A toner particle dispersion T-3 was obtained using the same method as in Example 1, but using octane (SP value=7.6) as the liquid a.

10 parts of the obtained toner particle dispersion T-3 was subjected to centrifugal separation; the supernatant was removed by decantation; replacement was carried out using fresh MT-30P in the same mass as the supernatant that had been removed; and 0.10 parts of hydrogenated lecithin (Lecinol S-10, Nikko Chemicals Co., Ltd.) was admixed as charge control agent to obtain the liquid developer of Example 3.

Examples 4 to 14 and Comparative Examples 1 to 11

20 Liquid Developer Production Example  
The liquid developers of Examples 4 to 14 and Comparative Examples 1 to 11 were obtained operating by the same method as described in the example of the synthesis of the liquid developer of Example 3, but changing to the parameters given in Table 6.

TABLE 6

| Example<br>No. | Polyester<br>resin A | Polyester<br>resin B | Toner particle<br>dispersing agent | B/<br>(A + B) | Production |          | Insulating<br>liquid carrier |
|----------------|----------------------|----------------------|------------------------------------|---------------|------------|----------|------------------------------|
|                |                      |                      |                                    |               | Procedure  | Liquid a |                              |
| 1              | PESA-1               | PESB- 1              | Dis-1                              | 0.4           | WP         | MT-30P   | MT-30P                       |
| 2              | PESA-1               | PESB- 1              | Dis-1                              | 0.4           | CO         | MT-30P   | MT-30P                       |
| 3              | PESA-1               | PESB- 1              | Dis-1                              | 0.4           | WP         | Octane   | MT-30P                       |
| 4              | PESA-1               | PESB- 1              | Dis-1                              | 0.8           | WP         | Octane   | MT-30P                       |
| 5              | PESA-1               | PESB- 1              | Dis-1                              | 0.3           | WP         | Octane   | MT-30P                       |
| 6              | PESA-1               | PESB- 1              | Dis-2                              | 0.3           | WP         | Octane   | MT-30P                       |
| 7              | PESA-2               | PESB- 1              | Dis-2                              | 0.3           | WP         | Octane   | MT-30P                       |
| 8              | PESA-2               | PESB- 2              | Dis-2                              | 0.3           | WP         | Octane   | MT-30P                       |
| 9              | PESA-3               | PESB- 2              | Dis-2                              | 0.3           | WP         | Octane   | MT-30P                       |
| 10             | PESA-3               | PESB-3               | Dis-2                              | 0.3           | WP         | Octane   | MT-30P                       |
| 11             | PESA-4               | PESB-4               | Dis-2                              | 0.3           | WP         | Octane   | MT-30P                       |
| 12             | PESA-5               | PESB-4               | Dis-2                              | 0.3           | WP         | Octane   | MT-30P                       |
| 13             | PESA-4               | PESB-5               | Dis-2                              | 0.3           | WP         | Octane   | MT-30P                       |
| 14             | PESA-4               | PESB-4               | Dis-2                              | 0.9           | WP         | Octane   | MT-30P                       |
| C.E. 1         | PESA-101             | PESB-4               | Dis-2                              | 0.3           | WP         | Octane   | MT-30P                       |
| C.E. 2         | PESA-102             | PESB-4               | Dis-2                              | 0.3           | WP         | Octane   | MT-30P                       |
| C.E. 3         | PESA-103             | PESB-4               | Dis-2                              | 0.3           | WP         | Octane   | MT-30P                       |
| C.E. 4         | PESA-104             | PESB-4               | Dis-2                              | 0.3           | WP         | Octane   | MT-30P                       |
| C.E. 5         | PESA-4               | PESB-101             | Dis-2                              | 0.3           | WP         | Octane   | MT-30P                       |
| C.E. 6         | PESA-4               | PESB-102             | Dis-2                              | 0.3           | WP         | Octane   | MT-30P                       |
| C.E. 7         | PESA-4               | PESB-103             | Dis-2                              | 0.3           | WP         | Octane   | MT-30P                       |
| C.E. 8         | PESA-4               | PESB-4               | Dis-101                            | 0.3           | WP         | Octane   | MT-30P                       |
| C.E. 9         | PESA-4               | PESB-4               | Dis-2                              | 1.0           | WP         | Octane   | MT-30P                       |
| C.E. 10        | PESA-4               | PESB-4               | Dis-2                              | 0.2           | WP         | Octane   | MT-30P                       |
| C.E. 11        | PESA-4               | PESB-4               | Dis-2                              | 0.3           | WP         | EtOH     | MT-30P                       |
| C.E. 12        | FC1565               | V220                 | PB817                              | 0.9           | CO         | P-40     | P-40                         |
| C.E. 13        | PESA-105             | PESB-104             | PB817                              | 0.4           | CO         | MT-30P   | MT-30P                       |

In Table 6, C. E. denotes Comparative Example; WP denotes Wet pulverization; CO denotes Coacervation; MT-30P denotes Moresco White MT-30P (Matsumura Oil Co., Ltd.); octane denotes n-octane; and EtOH denotes ethanol.

## Comparative Example 12

20.0 parts of MA285 (Mitsubishi Chemical Corporation), 8.0 parts of a pigment dispersing agent, and 72.0 parts of tetrahydrofuran (THF) were mixed and then kneaded for 15 minutes using a paint shaker and steel beads having a diameter of 5 mm. This was followed by kneading for an

IPA: isophthalic acid  
TMA: trimellitic anhydride

A urethane-modified polyester (PESB-104) was obtained by dissolving 100 parts of the resulting polyester resin in 300 parts of tetrahydrofuran, adding 10 parts of diphenylmethane diisocyanate, and reacting for 5 hours at 90° C. The property values of PESB-104 were a number-average molecular weight of 20,500 and an acid value of 0.9 mg KOH/g.

10 Comparative Example Resin PESA-105 Production Example

Polyester resin PESA-105, having the monomer molar proportions—as measured by NMR—given in Table 8, was synthesized by a known method.

TABLE 8

|          | BPA-EO | EG | NPG | TPA | IPA | TMA | Position of trimellitic anhydride | Mn    | SP value | Acid value |
|----------|--------|----|-----|-----|-----|-----|-----------------------------------|-------|----------|------------|
| PESA-105 | 10     | 0  | 0   | 9   | 0   | 1   | In main chain                     | 2,420 | 9.3      | 11.5       |

additional 2 hours using an Eiger Motor Mill M-250 (Eiger Japan Co., Ltd.) and zirconia beads having a diameter of 0.05 mm.

To 17.5 parts of the resulting kneaded material were added 21 parts of Vylon 220 (Toyobo Co., Ltd.), 3.5 parts of FC1565 (Mitsubishi Rayon Co., Ltd.), and 58 parts of THF and stirring was carried out with heating at 50° C. This was followed by the addition with stirring of 1.0 parts of the toner particle dispersing agent Ajisper PB817 (Ajinomoto Fine-Techno Co., Inc.), and a mixture was then prepared by stirring while diluting with 69.6 parts of Moresco White P-40 (Matsumura Petrochemical Laboratories Co., Ltd.).

Then, using a unit in which a solvent distillation apparatus (connected to a pressure-reduction unit) was connected to a homogenizer provided with a sealed stirred tank, the mixture was stirred at high speed (5,000 rpm) by the homogenizer and, while this was done, the pressure was reduced by the pressure-reduction unit so as to provide a mixture temperature of 50° C. The THF was completely distilled off from the sealed stirred tank to provide the liquid developer of Comparative Example 12.

## Comparative Example 13

## Comparative Example Resin PESB-104 Production Example

A polyester resin having the monomer mass proportions given in Table 7 was synthesized by a known method.

TABLE 7

|          | TPA | SIPA | NPG | PG | DPG | Mn    | Acid value<br>[mgKOH/g] |
|----------|-----|------|-----|----|-----|-------|-------------------------|
| PESB-104 | 43  | 1    | 4   | 36 | 8   | 1,400 | 0.5                     |

The following abbreviations are used in Table 7 and 8.

TPA: terephthalic acid

SIPA: monosodium 5-sulfoisophthalate

NPG: neopentyl glycol

PG: propylene glycol

DPG: dipropylene glycol

BPA-EO: 2 mol ethylene oxide adduct on bisphenol A

EG: ethylene glycol

## Liquid Developer Production Example

A kneaded material was obtained by mixing 30 parts of Pigment Blue 15:3, 15 parts of a 32% tetrahydrofuran solution of the urethane-modified polyester PESB-104, 15 parts of Ajisper PB-821 (Ajinomoto Fine-Techno Co., Inc.), 255 parts of tetrahydrofuran, and 130 parts of glass beads (1 mm Ø); carrying out dispersion for 3 hours using an attritor (Nippon Coke & Engineering Co., Ltd.); and filtration across a mesh.

18 parts of the obtained kneaded material, 12.6 parts of a 50% tetrahydrofuran solution of polyester PESA-105, and 35 2.1 parts of a toner particle dispersing agent (Ajisper PB-817, Ajinomoto Fine-Techno Co., Inc.) were mixed using a high-speed disperser (T. K. Robomix/T. K. Homodisper Model 2.5 blade, PRIMIX Corporation) and were mixed while stirring at 40° C. to obtain a colorant dispersion.

40 A mixture was obtained by adding 200 parts of Moresco White MT-30P (Matsumura Oil Co., Ltd.) in small portions to 100 parts of the obtained colorant dispersion while stirring at high speed (25,000 rpm) using a homogenizer (Ultra-Turrax T50, IKA).

45 The resulting mixture was transferred to a recovery flask and the tetrahydrofuran was completely distilled off at 50° C. while applying ultrasound dispersion to obtain a toner particle dispersion in which toner particles were dispersed in an insulating liquid carrier.

## Liquid Developer Preparation Step

50 10 parts of the resulting toner particle dispersion was subjected to a centrifugal separation treatment and the supernatant was removed by decantation. Fresh Moresco 55 White MT-30P was then added in the same mass as the supernatant that had been removed and the toner particle dispersion was redispersed. 0.10 parts of Lecinol S-10 (hydrogenated lecithin, Nikko Chemicals Co., Ltd.) was added to the resulting dispersion to yield the liquid developer of Comparative Example 13.

## Measurement and Evaluation of Toner Particle Dispersion Stability

55 Immediately after the production of the resulting liquid developer, a 2-hour continuous print run was carried out 60 using the image-forming apparatus shown in FIG. 1 and FIG. 2 (14,400 prints at 120 prints/minute of A4 size of the N7 natural image of "High-Definition Color Digital Stan-

dard Images (XYZ/SCID)" of JIS X 9204:2004). After the 2-hour continuous print run, the 50% particle diameter on a volume basis (D50) of the toner particle was measured using a laser diffraction/scattering particle size distribution analyzer (product name: "LA-950", Horiba, Ltd.). The ratio D50<sub>2h</sub>/D50<sub>0h</sub> was determined. The evaluation was performed based on this particle diameter increase ratio.

A D50<sub>2h</sub>/D50<sub>0h</sub> ratio of not greater than 2 was regarded as excellent.

The reference signs in the figures are as follows.

**10C, 10M, 10Y, 10K:** developer container; **11C:** film-production counterelectrode; **12C:** recovery unit; **13C, 13M, 13Y, 13K:** development liquid supply pump; **14C:** development liquid recovery pump; **20:** pre-wet roller; **21:** pre-wet counter roller; **30:** secondary transfer unit; **31:** secondary transfer roller; **40:** intermediate transfer belt; **41:** belt driving roller; **42:** driven roller; **50C, 50M, 50Y, 50K:** image-forming unit; **51C, 51M, 51Y, 51K:** developing unit; **52C, 52M, 52Y, 52K:** photosensitive member; **53C:** development roller; **54C:** concentration roller; **55C:** cleaning roller; **56C:** photoexposure unit; **57C:** charging unit; **58C:** static-eliminating unit; **59C:** recovery blade; **60C, 60M, 60Y, 60K:** primary transfer unit; **61C, 61M, 61Y, 61K:** primary transfer roller; **80:** recording medium; **90:** developer curing unit

The results of the evaluations for Examples 1 to 14 and Comparative Examples 1 to 13 are given in Table 9.

weight of the polyester resin A is not more than 7,000, after the durability test the particle diameter is not greater than 2  $\mu\text{m}$  and the particle diameter ratio is not greater than 2.0-fold and aggregation is thus inhibited.

5 The results for Example 12 and Comparative Example 3 demonstrate that, when the acid value of the polyester resin A is at least 5 mg KOH/g, after the durability test the particle diameter is not greater than 2  $\mu\text{m}$  and the particle diameter ratio is not greater than 2.0-fold and aggregation is thus inhibited.

10 The results for Example 11 and Comparative Example 4 demonstrate that, when the polyester resin A contains a carboxy group deriving from trimellitic acid or trimellitic anhydride as an acidic group, after the durability test the particle diameter is not greater than 2  $\mu\text{m}$  and the particle diameter ratio is not greater than 2.0-fold and aggregation is thus inhibited.

15 The results for Example 10 and Comparative Example 6 demonstrate that, when the number-average molecular weight of the polyester resin B is at least 4,000, after the durability test the particle diameter is not greater than 2  $\mu\text{m}$  and the particle diameter ratio is not greater than 2.0-fold and aggregation is thus inhibited.

20 The results for Example 13 and Comparative Example 5 demonstrate that, when the number-average molecular weight of the polyester resin B is not more than 20,000, after

TABLE 9

| Example No. | Liquid a       | Toner particle dispersing agent | Second term in formula (7) | Polyester resin B | Evaluation       |                      |                                      |
|-------------|----------------|---------------------------------|----------------------------|-------------------|------------------|----------------------|--------------------------------------|
|             |                |                                 |                            |                   | Initial D50 [nm] | durability test [nm] | D50 <sub>2h</sub> /D50 <sub>0h</sub> |
| 1           | 7.9            | 10.9                            | 11.2                       | 12.0              | 605              | 702                  | 1.2                                  |
| 2           | 7.9            | 10.9                            | 11.2                       | 12.0              | 604              | 664                  | 1.1                                  |
| 3           | 7.6            | 10.9                            | 11.2                       | 12.0              | 605              | 796                  | 1.3                                  |
| 4           | 7.6            | 10.9                            | 11.2                       | 12.0              | 599              | 802                  | 1.3                                  |
| 5           | 7.6            | 10.9                            | 11.2                       | 12.0              | 596              | 849                  | 1.4                                  |
| 6           | 7.6            | 10.6                            | 10.9                       | 12.0              | 604              | 896                  | 1.5                                  |
| 7           | 7.6            | 10.6                            | 10.9                       | 12.0              | 594              | 951                  | 1.6                                  |
| 8           | 7.6            | 10.6                            | 10.9                       | 12.0              | 607              | 1004                 | 1.7                                  |
| 9           | 7.6            | 10.6                            | 10.7                       | 12.0              | 596              | 1050                 | 1.8                                  |
| 10          | 7.6            | 10.6                            | 10.7                       | 12.0              | 597              | 1104                 | 1.9                                  |
| 11          | 7.6            | 10.6                            | 11.7                       | 11.4              | 603              | 1203                 | 2.0                                  |
| 12          | 7.6            | 10.6                            | 11.7                       | 11.4              | 595              | 1203                 | 2.0                                  |
| 13          | 7.6            | 10.6                            | 11.7                       | 11.4              | 600              | 1198                 | 2.0                                  |
| 14          | 7.6            | 10.6                            | 11.7                       | 11.4              | 607              | 1198                 | 2.0                                  |
| C.E. 1      | 7.6            | 10.6                            | 11.3                       | 11.4              | 1512             | 5593                 | 3.7                                  |
| C.E. 2      | 7.6            | 10.6                            | 10.5                       | 11.4              | 604              | 2194                 | 3.6                                  |
| C.E. 3      | 7.6            | 10.6                            | 10.9                       | 11.4              | 597              | 2192                 | 3.7                                  |
| C.E. 4      | 7.6            | 10.6                            | 10.9                       | 11.4              | 596              | 2191                 | 3.7                                  |
| C.E. 5      | 7.6            | 10.6                            | 11.7                       | 12.0              | 1295             | 4791                 | 3.7                                  |
| C.E. 6      | 7.6            | 10.6                            | 11.7                       | 12.0              | 599              | 2186                 | 3.7                                  |
| C.E. 7      | 7.6            | 10.6                            | 11.7                       | 12.0              | 593              | 2191                 | 3.7                                  |
| C.E. 8      | 7.6            | 10.2                            | 11.2                       | 11.4              | 597              | 2213                 | 3.7                                  |
| C.E. 9      | 7.6            | 10.6                            | 11.7                       | 11.4              | 606              | 2178                 | 3.6                                  |
| C.E. 10     | 7.6            | 10.6                            | 11.7                       | 11.4              | 606              | 2207                 | 3.6                                  |
| C.E. 11     | 14             | 10.6                            | 11.7                       | 11.4              | 2156             | 5999                 | 2.8                                  |
| C.E. 12     | Not determined |                                 |                            | 12.0              | 708              | 3098                 | 4.4                                  |
| C.E. 13     | 7.3            | Not determined                  | 11.7                       | 701               | 3099             | 4.4                  |                                      |

In Table 9, C. E. denotes Comparative Example.

The results for Examples 9 and 10 and Comparative Example 2 demonstrate that, when the number-average molecular weight of the polyester resin A is at least 3,000, after the durability test the particle diameter is not greater than 2  $\mu\text{m}$  and the particle diameter ratio is not greater than 2.0-fold and aggregation is thus inhibited.

The results for Example 11 and Comparative Example 1 demonstrate that, when the number-average molecular

60 the durability test the particle diameter is not greater than 2  $\mu\text{m}$  and the particle diameter ratio is not greater than 2.0-fold and aggregation is thus inhibited.

65 The results for Example 10 and Comparative Example 7 demonstrate that, when the acid value of the polyester resin B is not more than 5 mg KOH/g, after the durability test the particle diameter is not greater than 2  $\mu\text{m}$  and the particle diameter ratio is not greater than 2.0-fold and aggregation is thus inhibited.

35

The results for Example 11 and Comparative Example 8 demonstrate that, when the amine value of the toner particle dispersing agent is at least 40 mg KOH/g, after the durability test the particle diameter is not greater than 2  $\mu\text{m}$  and the particle diameter ratio is not greater than 2.0-fold and aggregation is thus inhibited.

The results for Examples 11 and 14 and Comparative Examples 9 and 10 demonstrate that, when the B/(A+B) mass ratio for the polyester resin A and the polyester resin B is from 0.3 to 0.9, after the durability test the particle diameter is not greater than 2  $\mu\text{m}$  and the particle diameter ratio is not greater than 2.0-fold and aggregation is thus inhibited.

The results for Example 11 and Comparative Example 11 demonstrate that, when the relationship: SP value of liquid a<SP value of the toner particle dispersing agent<SP value of polyester resin B is satisfied, after the durability test the particle diameter is not greater than 2  $\mu\text{m}$  and the particle diameter ratio is not greater than 2.0-fold and aggregation is thus inhibited.

A comparison of Example 11 with Example 10 demonstrates that, when the SP value of the polyester resin B and the SP value of the liquid a satisfy formula (7), the particle diameter ratio after the durability test goes from 2.0-fold to 1.9-fold and the aggregation-inhibiting effect is thus further increased.

A comparison of Example 9 with Example 10 demonstrates that, when the number-average molecular weight of the polyester resin B is made at least 7,000, the particle diameter ratio after the durability test goes from 1.9-fold to 1.8-fold and the aggregation-inhibiting effect is thus further increased.

A comparison of Example 8 with Example 9 demonstrates that, when the number-average molecular weight of the polyester resin A is made at least 4,000, the particle diameter ratio after the durability test goes from 1.8-fold to 1.7-fold and the aggregation-inhibiting effect is thus further increased.

A comparison of Example 7 with Example 8 demonstrates that, when the polyester resin B has a sulfo group that has formed a salt with at least one element selected from the alkali metals and alkaline-earth metals, the particle diameter ratio after the durability test goes from 1.7-fold to 1.6-fold and the aggregation-inhibiting effect is thus further increased.

A comparison of Example 6 with Example 7 demonstrates that, when the acidic group of the polyester resin A is present in terminal position on the polyester resin A, the particle diameter ratio after the durability test goes from 1.6-fold to 1.5-fold and the aggregation-inhibiting effect is thus further increased.

A comparison of Example 5 with Example 6 demonstrates that, when the amine value of the toner particle dispersing agent is at least 60 mg KOH/g, the particle diameter ratio after the durability test goes from 1.5-fold to 1.4-fold and the aggregation-inhibiting effect is thus further increased.

A comparison among Example 3, Example 4, and Example 5 demonstrates that, when the B/(A+B) mass ratio for the polyester resin A and the polyester resin B is from 0.4 to 0.8, the particle diameter ratio after the durability test goes from 1.4-fold to 1.3-fold and the aggregation-inhibiting effect is thus further increased.

A comparison of Example 1 with Example 3 demonstrates that, when an insulating liquid carrier is used as the liquid a, the particle diameter ratio after the durability test goes from 1.3-fold to 1.2-fold and the aggregation-inhibiting effect is thus further increased.

The results for Example 1 and Example 2 demonstrate that the particle diameter ratio after the durability test is brought to 1.1-fold—and the aggregation-inhibiting effect is thus further increased—through production of the toner particle by the so-called coacervation method.

36

The results for Comparative Example 12 demonstrated that the effects of the present invention are not obtained with the method described in the examples of Japanese Patent Application Laid-open No. 2014-232211, which is a method that does not satisfy claim 1 of the present invention.

The results for Comparative Example 13 demonstrated that the effects of the present invention are not obtained with the method described in the examples of Japanese Patent Application Laid-open No. 2016-224405, which is a method that does not satisfy claim 1 of the present invention.

### Example 15

Cationically Polymerizable, Ultraviolet-Curable Liquid Developer Production Example

Liquid Developer Production Example Using Coacervation Method

Pigment Dispersion Production Step

Pigment Dispersion Production Example

20 Pigment Blue 15:3 (30 parts), Vylon UR4800 (47 parts), 255 parts of tetrahydrofuran, and 130 parts of glass beads (1 mm Ø) were mixed; dispersion was performed for 3 hours using an attritor [Nippon Coke & Engineering Co., Ltd.]; and filtration across a mesh was carried out to obtain a kneaded material.

15 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680

## (Cationically Polymerizable, Ultraviolet-Curable Liquid Developer Production Example)

A cationically polymerizable, ultraviolet-curable liquid developer was obtained using the same method as in Example 16, but, as shown in Table 10, changing the liquid a to oxetane.

TABLE 10

| Liquid developer | Polyester resin A | Polyester resin B | Toner particle dispersing agent | B/ (A + B) | Production Procedure | Liquid a | Insulating liquid carrier |
|------------------|-------------------|-------------------|---------------------------------|------------|----------------------|----------|---------------------------|
| Example 15       | PESA-1            | PESB-1            | Dis-1                           | 0.4        | CO                   | DDVE     | UL                        |
| Example 16       | PESA-1            | PESB-1            | Dis-1                           | 0.4        | WP                   | DDVE     | UL                        |
| Example 17       | PESA-1            | PESB-1            | Dis-1                           | 0.4        | WP                   | OXT-221  | UL                        |

In Table 10, WP denotes Wet pulverization; CO denotes Coacervation; UL denotes Ultraviolet-Curable Liquid; DDVE denotes dodecyl vinyl ether (SP value=8.13); and OXT-221 denotes oxetane (SP value=8.8, Toagosei Co., Ltd.).

## Measurement and Evaluation of Toner Particle Dispersion Stability

Using the same method as for Examples 1 to 13 and Comparative Examples 1 to 13, the value of the 50% particle diameter on a volume basis (D50) was evaluated immediately after production of the liquid developer and after the two-hour durability test and the ratio between these values was evaluated.

## Evaluation of Fixing Performance of Cationically Polymerizable, Ultraviolet-Curable Liquid Developers

Operating in an environment at room temperature (25°C.) and a humidity of 50%, the ultraviolet-curable liquid developer was dripped onto a polyethylene terephthalate film (Teijin Limited, Panlite : PC-2151, thickness=0.3 mm); bar coating was carried out using a wire bar (No. 6) [supplier: Matsuo Sangyo Co., Ltd.] (the resulting film had a thickness of 8.0 µm); and a cured film was formed by irradiating light at a wavelength of 365 nm from a high-pressure mercury lamp having a lamp output of 120 mW/cm<sup>2</sup>. The irradiated light dose was measured at the point at which surface tack (stickiness) was absent and complete curing had occurred.

The evaluation was performed using the following criteria.

5: 100 mJ/cm<sup>2</sup>

4: 200 mJ/cm<sup>2</sup>

3: 400 mJ/cm<sup>2</sup>

2: 1,000 mJ/cm<sup>2</sup>

1: not cured at 2,000 mJ/cm<sup>2</sup>

All of the fixing performance ranks equal to or greater than 3 were regarded as passing.

The results of the evaluations for Examples 15 to 17 are given in Table 11.

TABLE 11

| Liquid developer | Liquid a | Toner particle dispersing agent | Second term in formula (7) | Polyester resin B | Evaluation      |                     |                                        |                          |
|------------------|----------|---------------------------------|----------------------------|-------------------|-----------------|---------------------|----------------------------------------|--------------------------|
|                  |          |                                 |                            |                   | Initial D50[nm] | durability test[nm] | D50 <sub>2 h</sub> /D50 <sub>0 h</sub> | Evaluation of durability |
| Example 15       | 8.1      | 10.9                            | 11.2                       | 12.0              | 498             | 500                 | 1.0                                    | 5                        |
| Example 16       | 8.1      | 10.9                            | 11.2                       | 12.0              | 595             | 650                 | 1.1                                    | 5                        |
| Example 17       | 8.8      | 10.9                            | 11.2                       | 12.0              | 606             | 697                 | 1.1                                    | 3                        |

The results for Example 17 demonstrate that, when a cationically polymerizable liquid monomer, such as a vinyl ether compound, was used for the insulating liquid carrier, a liquid developer having an excellent durability was obtained and the particle diameter ratio after durability testing was brought to 1.1-fold, thus further increasing the aggregation-inhibiting effect.

A comparison of Example 16 with Example 17 demonstrates that, when a vinyl ether compound and a compound with formula (8) are incorporated, a liquid developer with an excellent durability is obtained, which cures at an even lower energy, and in combination with this the particle diameter ratio after durability testing is brought to 1.1-fold, thus further increasing the aggregation-inhibiting effect.

A comparison of Example 15 with Example 16 shows that, by producing the toner particle by a so-called coacervation method, a liquid developer with an excellent durability is obtained, which cures at low energy, and in combination with this the particle diameter ratio after durability testing is brought to 1.0-fold, thus further increasing the aggregation-inhibiting effect.

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2017-222664, filed Nov. 20, 2017, and Japanese Patent Application No. 2018-129132, filed Jul. 6, 2018, which are hereby incorporated by reference herein in their entirety.

What is claimed is:

1. A method for producing a liquid developer containing an insulating liquid carrier, a toner particle dispersing agent, and a toner particle that contains a polyester resin A and a polyester resin B, the method comprising the following process A or process B:

the process A having  
a step of particulating a mixture of the polyester resin A, the polyester resin B, and the toner particle dispersing agent in a liquid a by applying a shear force to the mixture, and

39

a step of producing a toner particle in the liquid a via a molten state; and  
 the process B having  
 a step of dissolving, in a solvent b, a mixture of the polyester resin A, the polyester resin B, and the toner particle dispersing agent,  
 a step of mixing the resulting solution with the liquid a and applying a shear force to particulate the mixture in the liquid a and provide a toner particle, and  
 a step of distillatively removing the solvent b, wherein the liquid a dissolves the toner particle dispersing agent and does not dissolve the polyester resin A and does not dissolve the polyester resin B,  
 the polyester resin A has a number-average molecular weight from 3,000 to 7,000,  
 the polyester resin A has an acid value of at least 5 mg KOH/g,  
 the polyester resin A has, as an acidic group, a carboxy group deriving from trimellitic acid and/or trimellitic anhydride,  
 the polyester resin B has a number-average molecular weight from 4,000 to 20,000,  
 the polyester resin B has an acid value of not more than 2 mg KOH/g,  
 the toner particle dispersing agent has a primary amino group,  
 the toner particle dispersing agent has an amine value of at least 40 mg KOH/g,  
 a mass ratio (B/(A+B)) of the polyester resin B to a sum of the polyester resin A and the polyester resin B is from 0.3 to 0.9, and  
 an SP value of the liquid a, an SP value of the polyester resin B, and an SP value of the toner particle dispersing agent satisfy the following relationship: SP value of liquid a < SP value of toner particle dispersing agent < SP value of polyester resin B.

2. The method for producing a liquid developer according to claim 1, wherein the SP value of the polyester resin B and the SP value of the liquid a satisfy the following formula (7):

$$SP_{Caree} < \left( \frac{E_d + a \times n \times E_p}{V_d + a \times n \times V_p} \right)^{0.5} < SP_{PESB} \quad (7)$$

in formula (7), Ed and Ep respectively represent cohesive energy of the toner particle dispersing agent and the polyester resin A; Vd and Vp respectively represent a molar volume of the toner particle dispersing agent and the polyester resin A; a represents a number-average number of amino groups per molecule with respect to an average

40

degree of polymerization of the toner particle dispersing agent; n represents a number-average degree of polymerization of the polyester resin A; SP<sub>Caree</sub> represents the SP value of the liquid a; and SP<sub>PESB</sub> represents the SP value of the polyester resin B.

3. The method for producing a liquid developer according to claim 1, wherein the polyester resin B has a number-average molecular weight from 7,000 to 20,000.

4. The method for producing a liquid developer according to claim 1, wherein the polyester resin A has a number-average molecular weight from 4,000 to 7,000.

5. The method for producing a liquid developer according to claim 1, wherein the polyester resin B has a sulfo group that has formed a salt with at least one element selected from the group consisting of alkali metals and alkaline-earth metals.

6. The method for producing a liquid developer according to claim 1, wherein the carboxy group is present in terminal position on the polyester resin A.

20 7. The method for producing a liquid developer according to claim 1, wherein the toner particle dispersing agent has an amine value of at least 60 mg KOH/g.

8. The method for producing a liquid developer according to claim 1, wherein the mass ratio (B/(A+B)) of the polyester resin B to the sum of the polyester resin A and the polyester resin B is from 0.4 to 0.8.

9. The method for producing a liquid developer according to claim 1, wherein the liquid a is an insulating liquid carrier.

10. The method for producing a liquid developer according to claim 1, wherein the insulating liquid carrier contains a cationically polymerizable liquid monomer.

11. The method for producing a liquid developer according to claim 10, wherein the cationically polymerizable liquid monomer is a vinyl ether compound and the liquid developer contains a compound represented by the following formula (8):



in formula (8), R<sub>1</sub> and R<sub>2</sub> are bonded to each other to form a cyclic structure; x represents an integer from 1 to 8; and y represents an integer from 3 to 17.

\* \* \* \* \*